

## [54] STABILIZED SLURRY AND PROCESS FOR PREPARING SAME

[75] Inventor: James E. Funk, Alfred Station, N.Y.

[73] Assignee: Alfred University Research Foundation, Inc., Alfred Station, N.Y.

[\*] Notice: The portion of the term of this patent subsequent to Apr. 10, 2001 has been disclaimed.

[21] Appl. No.: 532,909

[22] Filed: Sep. 16, 1983

## Related U.S. Application Data

[63] Continuation-in-part of Ser. No. 474,125, Mar. 10, 1983, which is a continuation-in-part of Ser. No. 375,183, May 5, 1982, Pat. No. 4,441,887, which is a continuation-in-part of Ser. No. 288,737, Jul. 31, 1981, Pat. No. 4,416,666, which is a continuation-in-part of Ser. No. 088,815, Oct. 26, 1979, Pat. No. 4,282,006, which is a continuation-in-part of Ser. No. 957,166, Nov. 2, 1978, abandoned, which is a continuation-in-part of Ser. No. 790,337, Apr. 25, 1977, abandoned.

[51] Int. Cl. 3 ..... C10L 1/32

[52] U.S. Cl. ..... 44/51

[58] Field of Search ..... 44/51

## [56] References Cited

## U.S. PATENT DOCUMENTS

4,104,035 8/1978 Cole et al. ..... 44/51  
4,282,006 4/1981 Funk ..... 44/51Primary Examiner—Y. Harris Smith  
Attorney, Agent, or Firm—Howard J. Greenwald

## [57] ABSTRACT

A process for preparing a carbonaceous slurry with a Brookfield viscosity of less than 5,000 centipoise when it is measured at a solids content of 70 volume percent, ambient temperature, ambient pressure, and 100 revolutions per minute, is disclosed. In the first step of this process, a specified carbonaceous compact is provided which has a certain particle size distribution, a specific surface area of from about 0.8 to about 4.0 square meters per cubic centimeter, an interstitial porosity of less than about 20 volume, and which contains at least about 5 weight percent of colloidally sized carbonaceous particles and at least 85 weight percent of particles smaller than 300 microns. In the second stage of this process, from about 60 to about 80 parts, by volume, of said carbonaceous compact is mixed with from about 20 to about 40 parts, by volume, of carrier liquid, wherein (1) at least two liquids are mixed with said carbonaceous compact, (2) at least about 90 weight percent of the total amount of liquid mixed with said carbonaceous compact is water, and (3) no more than about 10 weight percent of the total amount of liquid mixed with said carbonaceous compact is non-aqueous liquid.

A carbonaceous slurry which contains from about 60–80 volume percent of carbonaceous solid material, which has a Brookfield viscosity at 70 volume percent solids of less than 5,000 centipoise, which contains said carbonaceous compact, which contains from about 20–40 volume percent of liquid wherein (1) at least two liquids are present in the slurry, (2) at least about 90 weight percent of the liquid in the slurry is water, and (3) no more than about 10 weight percent of the liquid in the slurry is non-aqueous liquid, also is disclosed.

13 Claims, 2 Drawing Figures





FIG. 1



FIG. 2

**STABILIZED SLURRY AND PROCESS FOR  
PREPARING SAME**

**CROSS-REFERENCE TO RELATED  
APPLICATIONS**

This application is a continuation-in-part of applicant's copending application U.S. Ser. No. 474,125 filed Mar. 10, 1983, which was a continuation-in-part of application Ser. No. 375,183 filed May 5, 1982 (now U.S. Pat. No. 4,441,887), which was a continuation-in-part of application Ser. No. 288,737 filed July 31, 1981 (now U.S. Pat. No. 4,416,666), which was a continuation-in-part of application Ser. No. 088,815 filed Oct. 26, 1979 (now U.S. Pat. No. 4,282,006), which was a continuation-in-part of application Ser. No. 957,166 filed Nov. 2, 1978 (now abandoned), which was a continuation-in-part of application Ser. No. 790,337 filed Apr. 25, 1977 (now abandoned).

**TECHNICAL FIELD**

A stabilized slurry containing carbonaceous solid material (such as coal or coke), at least two carrier liquids, and dispersing agent is disclosed. Also disclosed is a method of preparing said slurry by mixing carbonaceous material, said carrier fluids, and said dispersing agent; the reagents used and the mixing conditions are such that the slurry produced has a viscosity of less than about 5,000 centipoise at a solids content of 70 volume percent.

**BACKGROUND OF THE INVENTION**

U.S. Pat. No. 4,282,006 discloses a high-solids content, low-viscosity slurry comprised of carbonaceous solid material (such as coal) and liquid, which slurry can be pumped like a liquid and burned in a manner similar to the way oil is burned. The vast deposits of coal in the United States, the fact that such a coal-liquid slurry might be substantially cheaper than an equivalent amount of oil, and the need for the United States to reduce its dependence upon foreign oil indicate that such a slurry might be very important to this nation's economy.

Ideally, a slurry containing carbonaceous material and liquid should be stable under the dynamic conditions it might encounter during pumping and shipping. In the transportation of such a slurry, (such as by barge, marine tanker, rail car, or truck tank car) various stresses might be encountered. The vibrations the slurry will be subjected to will vary in both amplitude and frequency. Thus, for example, during shipboard travel when there is relatively little clearance between the hull and the harbor or river bottom, severe shaking of the ship will be caused by pressure waves from the ship's propellers. When shipboard travel occurs on the open water, by comparison, there will be more roll, and some pitch, but the amount of high frequency vibration should be relatively small. The amount of motion a slurry is subjected to during any type of travel should vary with the extent of confinement of the slurry: full tanks would slosh very little, and partially empty tanks would slosh considerably more.

One problem encountered with many prior art coal-water slurries is that they become unmixed when they are subjected to vibration, with disastrous consequences. When such a slurry is being pumped, the solid particles settle out of the slurry to the bottom of the pipe, thereby changing the solids content and other

properties of the slurry, clogging the pipe, and impeding the fluid flow of the slurry; often a hard pack of solid material is formed which is difficult or impossible to readily resuspend in the slurry.

5 It is probable that, to some extent, some settling will occur in coal-liquid slurries subjected to vibratory conditions. It is desirable to minimize the degree of settling. It is also desirable to provide a slurry wherein, even if settling does occur, the settled particles predominantly form a "soft pack" (as opposed to a hard pack) and can be easily resuspended in the slurry.

10 It is an object of this invention to provide a high-solids content slurry with low viscosity comprised of carbonaceous material and liquid which has improved stability properties. It is another object of this invention to provide a process for preparing said slurry.

**SUMMARY OF THE INVENTION**

15 20 A process for preparing a carbonaceous slurry with a Brookfield viscosity of less than 5,000 centipoise when it is measured at a solids content of 70 volume percent, ambient temperature, ambient pressure, and 100 revolutions per minute, is disclosed. In the first step of this process, a specified carbonaceous compact is provided which has a certain particle size distribution, a specific surface area of from about 0.8 to about 4.0 square meters per cubic centimeter, an interstitial porosity of less than about 20 volume, and which contains at least about 5 weight percent of colloidally sized carbonaceous particles and at least 85 weight percent of particles smaller than 300 microns. In the second stage of this process, from about 60 to about 80 parts, by volume, of said carbonaceous compact is mixed with from about 20 to about 40 parts, by volume, of carrier liquid, wherein (1) at least two liquids are mixed with said carbonaceous compact, (2) at least about 90 weight percent of the total amount of liquid mixed with said carbonaceous compact is water, and (c) no more than about 10 weight percent of the total amount of liquid mixed with said carbonaceous compact is non-aqueous liquid.

25 30 35 40 45 A carbonaceous slurry which contains from about 60-80 volume percent of carbonaceous solid material, which has a Brookfield viscosity at 70 volume percent solids of less than 5,000 centipoise, which contains said carbonaceous compact, which contains from about 20-40 volume percent of liquid wherein (1) at least two liquids are present in the slurry, (2) at least about 90 weight percent of the liquid in the slurry is water, and (3) no more than about 10 weight percent of the liquid in the slurry is non-aqueous liquid, also is disclosed.

**DETAILED DESCRIPTION OF THE  
DRAWINGS**

The present invention will be more fully understood by reference to the following detailed description hereof, when read in conjunction with the attached drawings, wherein like reference numbers refer to like elements and wherein:

55 FIG. 1 is a flow sheet of a preferred process for making the stabilized slurry of this invention, and

60 FIG. 2 is a chart showing the correlation between the zeta potential of coal particles in a fluid and the specific conductance of the fluid as a function of percent dispersing agent added to the fluid for two candidate dispersants.

DETAILED DESCRIPTION OF THE  
INVENTION

The Brookfield viscosity of the slurry produced by the process of this invention is less than about 5,000 centipoise; the Brookfield viscosity is tested after the solids concentration of the slurry is adjusted to a solids content of 70 volume percent (the slurry is either diluted or concentrated until it has this concentration of solids) at ambient temperature, ambient pressure, and a shear rate of 100 revolutions per minute. It is preferred that the viscosity of said slurry be less than 4,000 centipoise. It is more preferred that the viscosity of said slurry be less than 3,000 centipoise. In an even more preferred embodiment, the viscosity of the slurry is less than 2,000 centipoise. In the most preferred embodiment, the viscosity of the slurry is less than about 1,000 centipoise.

In the first step of the process of this invention, a carbonaceous compact with specified properties is provided. This carbonaceous compact is comprised of at least one carbonaceous solid material. As used in this specification, the term "carbonaceous" refers to a carbon-containing material and includes, by way of illustration and not limitation, coal, coke, graphite, charcoal, char, and the like. The preferred carbonaceous materials are carbonaceous fuels.

In one preferred embodiment, the carbonaceous solid is coal. By way of illustration, anthracite, semi-anthracite, medium, and high-volatile bituminous, sub-bituminous and lignite coals may advantageously be used to practice the invention.

The coal for use in the process can be obtained in a dry or wet form and mixed with fluid to form a coal-fluid mixture. Preferably, the coal for making a fine particle sized fraction is wet milled in known ways to prevent dust and explosion hazards, while optionally adding dispersing agent(s) to the fluid. The wet milled coal fraction can be milled with all the water, or it can be mixed with sufficient additional water to make a slurry when it is further mixed with a coarser crushed coal fraction.

In view of the manner in which coal fractures during milling, coal particles will have irregular shapes which, however, are of a body (or maximum side-to-side thickness) such that the sub-sieve sized discrete particles will pass through a specified mesh of a sieve. The size of the discrete particle can be expressed in terms of a spherical diameter which, as used herein, is defined as a U.S. sieve size of from 4 mesh (4760  $\mu\text{m}$ ) to 400 mesh (38  $\mu\text{m}$ ) through which a coal particle from a sample of coal or coal-water slurry will pass. For particles finer than 200 mesh (74  $\mu\text{m}$ ), the size of the particles can be determined by means of a sieve, or a sedimentometer, or a scanning electron microscope (SEM), or the like.

In one preferred embodiment, the carbonaceous solid material is coke. Coke is the solid, cellular, infusible material remaining after the carbonization of coal, pitch, petroleum residues, and certain other carbonaceous materials. The varieties of coke, other than those from coal, generally are identified by prefixing a word to indicate the source, e.g., "petroleum coke". To indicate the process by which a coke is manufactured, a prefix also is often used, e.g., "beehive coke".

High temperature coke can be used in this invention. As is known to those skilled in the art, this coke can be prepared from bituminous coal. Most of this type of coke is made in slot-type recovery ovens. In general,

5 this type of coke contains from about 0.6 to about 1.4 weight percent of volatile matter and has an apparent specific gravity of from about 0.8 to about 0.99.

6 Foundry coke can also be used in this invention. In general, the volatile matter in this type of coke is less than about 2 weight percent.

7 Low temperature coke and medium temperature coke can also be used in this invention.

8 Pitch coke can be used in this invention. Pitch coke is made from coal-tar pitch; it has about 1.0 percent volatile matter, and it generally contains less than 0.5 percent sulfur.

9 Petroleum coke can be used in this invention. There are at least two types of petroleum coke: delayed coke and fluid coke. Delayed coke generally contains from about 8 to about 18 weight percent volatile matter, has a grindability index of from about 40 to about 60, and has a true density of from about 1.28 to about 1.42 grams per milliliter. Fluid coke generally contains from about 3.7 to about 7.0 weight percent of volatile matter, has a grindability index of from about 20 to about 30, and has a true density of from about 1.5 to about 1.6 grams per milliliter.

10 In another preferred embodiment, the carbonaceous solid material is char. Char is the non-agglomerated, non-fusible residue from the thermal treatment of solid carbonaceous materials. Coal char is obtained as a residue or a coproduct from low-temperature carbonization processes; such a char typically contains from about 1 to about 5 weight percent of volatile matter.

11 In another preferred embodiment, the carbonaceous material is charcoal. Charcoal is the residue remaining after the destructive distillation of wood.

12 In yet another embodiment, the carbonaceous material is solvent refined coal.

13 In general, any carbonaceous fuel can be used as the solid carbonaceous material in this invention.

14 Mixtures of carbonaceous solids also can be used. By way of illustration and not limitation, one can use a mixture of at least one coarse carbonaceous fraction which contains less than about 30 weight percent of volatilizable hydrocarbons (such as, e.g., anthracite or low volatile bituminous coal) and at least one fine carbonaceous fraction which contains more than about 35 weight percent of volatilizable hydrocarbons (such as, e.g., lignite or high volatile bituminous coal). One can use a mixture of two or more of said coarse carbonaceous fractions and one of said fine fractions, one of said coarse carbonaceous fractions and two or more of said fine fractions, or two or more of said coarse carbonaceous fractions and two or more of said fine fractions.

15 In one of the embodiments of this invention, the slurry produced by mixing the carbonaceous compact with carrier liquid contains at least two consists of carbonaceous material. The term "consist", as it is used in this specification, and in the prior art, means the particle size distribution of the solid phase of the carbonaceous material/fluid slurry. For example, in the prior art, the term "8 mesh  $\times$  0", when used with reference to a coal-water slurry, indicates coal with a graded size, or consist, of coal particles distributed in the range of 8 mesh and zero, or 2360 microns  $\times$  zero microns. Similarly, the term "about 1180 microns  $\times$  0.05 microns" indicates coal with a nominally measurable graded size, or "consist", of coal particles distributed in the range of from about 1180 microns to a measurable colloidal size, e.g., at least about 0.05 microns. The term "about 1180 microns" is nominally equivalent to a U.S. Series 16 mesh

sieve, substantially as defined in "Handbook of Chemistry and Physics", 54th Edition, 1973-1974, CRC Press, Cleveland, Ohio, page 143, "Standard Test Sieves (wire cloth)", the disclosure of which is hereby incorporated by reference into this specification. Unless otherwise stated in this specification, the weight of carbonaceous material is on a moisture-free or "dry basis" herein. Thus, e.g., the "solids" in as-mined carbonaceous material include, e.g., carbonaceous material and ash. Thus, there is a considerable amount of bound water in coal as mined; the volume of this water in the coal is not included in the solids weight in order to calculate the volume percent of "dry solids" in the grinding mixture used in the process of this invention. Thus, as used herein, the term "dry basis" refers to coal (and/or other carbonaceous material) which is substantially free of carrier liquid. Carbonaceous material is considered to be dry after it has been air dried by being exposed to air at a temperature of at least 70 degrees Fahrenheit and a relative humidity of less than 50 percent for at least 24 hours.

In the first step of the process of this invention, a carbonaceous compact with a specified particle size distribution is provided. The term "compact", as used in this specification, refers to a mass of finely-divided particles which are closely packed in accordance with the CPFT formula described below. The particle size distribution of the compact provided in the process of this invention is substantially in accordance with the following formula:

$$\frac{CPFT}{100} = \sum_{j=1}^k \left[ X_j \left( \frac{D^{Nj} - D_{sj}^{Nj}}{D_{Lj}^{Nj} - D_{sj}^{Nj}} \right) \right]$$

where  $\sum_{j=1}^k X_j = 1.0$

and where if  $D < D_{sj}$   $\left( \frac{D^{Nj} - D_{sj}^{Nj}}{D_{Lj}^{Nj} - D_{sj}^{Nj}} \right) = 0.0$

and where if  $D > D_{Lj}$   $\left( \frac{D^{Nj} - D_{sj}^{Nj}}{D_{Lj}^{Nj} - D_{sj}^{Nj}} \right) = 1.0$

wherein:

1. CPFT is the cumulative percent of said solid carbonaceous material finer than a certain specified particle size  $D_s$  in volume percent;
  2.  $k$  is the number of component distributions in the consist and is at least 1;
  3.  $X_j$  is the fractional amount of the component  $j$  in the consist, is less than or equal to 1.0, and the sum of all of the  $X_j$ 's in the consist is 1.0;
  4.  $n$  is the distribution modulus of fraction  $j$  and is greater than about 0.001;
  5.  $D$  is the diameter of any particle in the consist and ranges from about 0.05 to about 1180 microns;
  6.  $D_s$  is the diameter of the particle in fraction  $j$ , measured at 1% CPFT on a plot of CPFT versus size  $D$ , is less than  $D_L$ , and is greater than 0.05 microns; and

7.  $D_L$  is the diameter of the size modulus in fraction j, measured by sieve size or its equivalent, and is from about 10 to about 1180 microns.

In the aforementioned CPFT formula,  $k$  is from about 1 to about 30, and most preferably is 1;  $X_j$  is the fractional amount of the component  $j$  in the consist, is less than or equal to 1.0, and the sum of all  $X_j$ 's in the consist is 1.0;  $n$  is the distribution modulus of fraction  $j$ , is greater than about 0.001, preferably is from about 0.001 to about 10.0 and more preferably from 0.01 to about 1.0, and most preferably is from about 0.01 to about 0.5;  $D$  is the diameter of any particle in the consist and ranges from about 0.05 to about 1180 microns;  $D_s$  is the diameter of the smallest particle in fraction  $j$  (as measured by extrapolating the CPFT chart line, if necessary, to one percent CPFT using data from sieve analyses plus the Micromeritics Sedigraph 5500L) and is generally greater than 0.05 microns but is less than  $D_L$ ;

$D_L$  represents the diameter of the largest particle in fraction  $j$  (sieve size or its equivalent), it ranges from about 10 to about 1180 microns, preferably is from about 30 to about 420 microns, and most preferably is from about 100 to about 300 microns;  $D_L$  is the theoretical size modulus of the particle size distribution; when CPFT is plotted against size, the  $D_L$  value is indicated as the intercept on the upper X axis of the CPFT/D plot. However, as is known to those skilled in the art, because of aberrations in grinding the coarse end of a particle size distribution, the actual top particle size is always larger than the  $D_L$  obtained by, e.g., the particle size equation described in this case; thus, e.g., a  $D_L$  size modulus of 250 microns will usually produce a particle distribution with at least about 98 percent of the particles smaller than 300 microns. Consequently, slurry has a compact with a particle size distribution which is substantially in accordance with the CPFT equation; minor deviations caused by the actual top size being greater than the  $D_L$  are within the scope and spirit of this invention.

When  $k$  is 1, the aforementioned equation simplifies to:

$$45 \quad \frac{CPFT}{100} = \frac{D^n - D_s^n}{D_L^n - D_s^n}$$

when  $k$  is 2, the equation becomes:

$$50 \quad \frac{CPFT}{100} = X_1 \left( \frac{D^{N1} - D_{s1}^{N1}}{D_{L1}^{N1} - D_{s1}^{N1}} \right) + X_2 \left( \frac{D^{NL} - D_{s2}^{N2}}{D_{L2}^{N2} - D_{s2}^{N2}} \right)$$

wherein:  $X_1 + X_2 = 1.0$  (i.e., the sum of the fractional parts is equal to the whole); when  $D$  is less than or equal to  $D_{S1}$ , the first term in the parentheses (term I) is equal to 0.0; when  $D$  is greater than or equal to  $D_{L1}$ , the first term in the parentheses (term I) is equal to 1.0; when  $D$  is less than  $D_{S2}$ , the second term in the parentheses (term II) is equal to 0.0; when  $D$  is greater than  $D_{L2}$ , the second term in the parentheses (term II) is equal to 1.0.

65 The reason for the aforementioned constraints of the terms in parentheses I and II is that each of these terms refers to the equation of one of the two components.

In order to sum the fractional parts of the two component distributions, the above considerations must be

included since particles of a certain size may be represented between the effective  $D_s$  and  $D_L$  of the total distribution but not between the  $D_s$  or  $D_L$  of one of the component distributions. Thus, the values in parentheses I and II are subject to the limitations that, when  $D$  is less than or equal to  $D_s$ , the value for the term is 0.0 and when  $D$  is greater than  $D_L$ , the value of the term is 1.0.

The equation given above for when  $k$  is 2 is simply the sum of two components where the fraction of component  $j_1$  is  $X_1$  and the fraction of component  $j_2$  is  $X_2$ . Since, in this case,  $X_1$  and  $X_2$  make up the whole distribution, their sum must equal 1.0.

In accordance with the above reasoning, when  $k=3$ , the equation becomes:

$$\frac{CPFT}{100} = X_1 \left( \frac{D^{N_1} - D_{s1}^{N_1}}{D_{L1}^{N_1} - D_{s1}^{N_1}} \right) + X_2 \left( \frac{D^{N_2} - D_{s2}^{N_2}}{D_{L2}^{N_2} - D_{s2}^{N_2}} \right) + X_3 \left( \frac{D^{N_3} - D_{s3}^{N_3}}{D_{L3}^{N_3} - D_{s3}^{N_3}} \right)$$

When  $k=4$ , there is a fourth term in the equation equal to

$$X_4 \left( \frac{D^{N_4} - D_{s4}^{N_4}}{D_{L4}^{N_4} - D_{s4}^{N_4}} \right)$$

In the first step of the process of this invention, a carbonaceous compact with a specified particle size distribution and specific surface area is provided. The compact has a specific surface area of from about 0.8 to about 4.0 square meters per cubic centimeter. It is preferred that said specific surface area be from about 0.8 to about 3.0 square meters per cubic centimeter and, more preferably, from about 0.8 to about 2.4 square meters per cubic centimeter. In the most preferred embodiment, said specific surface area is from about 0.8 to about 2.0 square meters per cubic centimeter.

As used in this specification, the term "specific surface area" refers to the summation of the surface area of equivalent spheres in the particle size distribution as measured by sieve analysis and sedimentation techniques; the particle size distribution of the consist in the slurry is first determined, it is assumed that all particles are spherical, and then one calculates the surface area based on this assumption.

For any given compact, one can determine the particle size distribution by means well known to those skilled in the art. For measuring particle sizes and for determining particle size distributions of pulverized and fine grind carbonaceous particles used for preparing a carbonaceous slurry, the following two means of measuring particle sizes can be used and are preferred:

1. U.S. Series sieves Nos. 16, 20, 30, 40, 50, 70, 100, 140, 200, 270, are used to determine weights of carbonaceous particles passing through each sieve in the range

of about  $(-)$  1180  $\mu\text{m}$  to  $(-)$  53  $\mu\text{m}$ . The cumulative volume percents of particles, dry basis, finer than (CPFT) a particular stated sieve size in microns is charted against the sizes in microns on a log-log chart, referred to herein as a "CPFT chart", to indicate the nature of the particle size distribution of 16 mesh  $\times$  270 mesh particles.

2. A Sedigraph 5500L (made by Micromeritics, Co., Norcross, Ga., U.S.) is used to measure particle sizes and numbers of particles in the carbonaceous material and in the slurry in the range of  $(-)$  75  $\mu\text{m}$  to about 0.2 mm. The Sedigraph 5500L uses photo-extinction of settling particles dispersed in water according to Stoke's law as a means for making the above determinations. Other instruments, such as a Coulter Counter or combinations of the Leeds & Northrup Microtrac Particle Analyzers can also be used for similar accuracy. The results can be plotted on a CPFT chart. Although these data do not necessarily extend to the size axis at 1% CPFT, the " $D_s$  at 1%" can be determined by extrapolating the CPFT chart line to this axis and reading the intercept. This number, although not the true  $D_s$ , can be effectively used in the computer algorithm to determine % porosity and specific surface area.

In addition to the above methods, particle size measurements can be estimated from methylene blue index measurements to obtain an approximate determination of the wgt. % of colloidal particles of size below 1 mm. Such a procedure is described in A.S.T.M. Standard C837-76. This index can be compared with the surface area calculated by the CPFT algorithm.

Once the particle size distribution of the consist is determined, it is assumed that each particle in the consist is spherical with a surface area of  $\pi D^2$ ; the diameter  $D$  of the particles in each class of particles in the consist is known; and the surface area of the particles in each class is calculated and summed.

The compact provided in the first step of the process of this invention has an interstitial porosity of less than about 20 volume percent. Said interstitial porosity is preferably less than about 15 volume percent and, even more preferably, less than about 10 volume percent. The interstitial porosity is a function of the volume between the interstices of the particles in the compact. For any given space full of particles, the interstitial porosity is equal to the "minimum theoretical porosity" in accordance with the equation presented below.

$$\text{Minimum Theoretical Porosity} = 40\% (1 - [1/VA])$$

where VA is as defined by the following modified Westman-Hugill algorithm:

$$\begin{aligned} VA_1 &= A_1 X_1 \\ VA_2 &= X_1 + A_2 X_2 \\ VA_3 &= X_1 + X_2 + A_3 X_3 \\ &\vdots \\ VA_i &= \sum_{j=1}^{i-1} X_j + A_i X_i \\ &\vdots \\ VA_n &= \sum_{j=1}^{n-1} X_j + A_n X_n \end{aligned}$$

wherein:

$A_i$ =Apparent volume of a monodispersion of the  $i^{\text{th}}$  size particle,

$X_i$ =Mass fraction of the  $i^{\text{th}}$  size particles,

$VA_i$ =Apparent volume calculated with reference to the  $i^{\text{th}}$  size particles,

$n$ =Number of particle sizes, and

$VA$ =Maximum value of  $VA_i$ =Apparent volume of the mixture of  $n$  particle sizes.

To determine the interstitial porosity of any compact, the particle size distribution of said compact can be determined by the method described above with reference to the measurement of the specific surface area. Thereafter it is assumed that each particle in the compact is spherical, the volume of the particles is calculated in accordance with this assumption, and the interstitial porosity of the compact is calculated in accordance with the above formula. It should be noted that this calculated porosity is less than the true porosity of the compact as measured, for example, by liquid less—due to the non-spherical morphology (shape) of the particles, and by invocation of  $D_s$  at 1%.

The carbonaceous compact provided in the first step of the process of this invention is comprised of at least about 5 weight percent of colloidal carbonaceous particles and, preferably, from about 5 to about 70 weight percent of said colloidal particles. As is used herein, the term "colloidal" refers to a substance of which at least one component is subdivided physically in such a way that one or more of its dimensions lies in the range of 100 angstroms and 3 microns. As is known, these are not fixed limits and, occasionally, systems containing larger particles are classified as colloids. See *Encyclopedia of Chemistry*, 2d Edition, Clark et al (Reinhold, 1966), page 203, the disclosure of which is hereby incorporated herein by reference.

It is preferred that, in the carbonaceous compact, at least 5 weight percent of the carbonaceous particles are smaller than about 3.0 microns. It is preferred that from about 5 to about 70 weight percent of the carbonaceous particles be smaller than 3.0 microns. In one preferred embodiment, from about 5 to about 30 weight percent of the carbonaceous particles are smaller than 3.0 microns. In another preferred embodiment, from about 7 to about 20 weight percent of the particles are smaller than 3.0 microns.

The compact provided in the first step of the process of this invention preferably has a substantial number of particles smaller than 300 microns. It is preferred that at least 85 weight percent of the carbonaceous particles in said compact have a particle size less than 300 microns. It is more preferred that at least 90 weight percent of the carbonaceous particles in the compact are smaller than 300 microns. In the most preferred embodiment, at least 95 weight percent of the carbonaceous particles in the compact are smaller than 300 microns.

The process of this invention involves the steps of (1) providing the aforementioned carbonaceous compact, and (2) mixing said carbonaceous compact with liquid. In one embodiment, step (1) is done prior to step (2). In another embodiment, step (1) is done simultaneously with step (2).

In one embodiment of this invention, the carbonaceous compact is provided prior to the time it is mixed with the liquid. Thus, e.g., one or more carbonaceous materials may be dry ground, until a compact is produced with the specified particle properties. Thus, e.g., one or more carbonaceous materials may be dry blended until a compact is produced with the specified

particle properties. Thus, e.g., one or more carbonaceous materials can be dry ground and dry blended in one or more steps to produce a compact with the desired properties.

In another embodiment of this invention, the carbonaceous compact is provided at the same time it is mixed with the amount of liquid required to produce a slurry containing 60-80 volume percent of solids. In this embodiment, from about 60 to about 80 parts (by volume) of carbonaceous material is mixed with from about 20 to about 40 parts (by volume) of carrier liquid, and the carbonaceous compact is formed during the time the solid material is mixed with the liquid. In one aspect of this embodiment, the carbonaceous material is mixed with the liquid, and the resulting grinding mixture is wet ground until a carbonaceous compact (or consist) which has the required particle and physical properties is formed in situ. In another aspect of this embodiment, one or more carbonaceous materials is mixed with the carrier liquid and wet ground, and thereafter one or more additional carbonaceous fractions, in either dry or wet form, is added to the mixture to form the desired compact in situ. Other aspects of this embodiment, which involve forming the compact in situ while either grinding and/or blending carbonaceous material while it is in contact with carrier liquid, will be apparent to those skilled in the art; and they are intended to be comprehended within the scope of this invention.

As used in this specification, the terms "mixed" and "mixing" refer to the steps of combining or blending several masses into one mass and includes, e.g., blending, grinding, milling, and all other steps by which two or more masses are brought into contact with each other and combined to some extent. Conventional means for mixing viscous materials can be used in the process of this invention. Thus, by way of illustration and not limitation, one can use batch mixers such as

change-can mixers, stationary tank mixers, gate mixers, shear-bar mixers, helical blade mixers, double-arm kneading mixers, screw-discharge batch mixers, intensive mixers, roll mills, bulk blenders, Littleford-Lodige mixers, cone and screw mixers, pan muller mixers, and the like; one can use continuous mixers such as single-screw extruders, the Rietz extruder, the Baker Perkins Ko-Kneader, the Transfer-Mix, the Baker Perkins Rotofeed, twin-screw continuous mixers, trough and screw mixers, pug mills, the Kneadermaster, and the like.

In the process of this invention, from about 60 to about 80 parts, by volume, of said carbonaceous compact are mixed with from about 20 to about 40 parts, by volume, of liquid. It is preferred to mix from about 65 to about 80 parts, by volume, of the compact, with from about 20 to about 35 parts, by volume, of liquid. In the most preferred embodiment, from about 70 to about 80 parts, by volume, of the compact, is mixed with from about 20 to about 30 parts, by volume, of the liquid.

In the process of this invention, the liquid mixed with the carbonaceous compact is comprised of at least two separate liquids. At least one of the liquids so mixed is water, and at least about 90 weight of the total amount of liquid mixed with the compact is water. It is preferred that at least about 95 weight percent of the total amount of the liquid mixed with the compact is water, and it is more preferred that at least about 97 weight percent of the total amount of the liquid mixed with the compact is water. In the most preferred embodiment, at

least about 98 weight percent of the total amount of liquid mixed with the compact is water.

As stated above, at least two liquids are mixed with the carbonaceous compact. At least one of the liquids so mixed is water, and at least one of the liquids so mixed is a non-aqueous liquid. From about 0.1 to about 10.0 weight percent, by weight of the total amount of the liquid mixed with the compact, is non-aqueous liquid. It is preferred that from about 0.2 to about 5.0 weight percent, by weight of the total amount of liquid mixed with the compact, be non-aqueous liquid. It is more preferred that from about 0.3 to about 3.0 weight percent, by weight of the total amount of liquid mixed with the compact, be non-aqueous liquid. In the most preferred embodiment, from about 0.4 to about 2.0 weight percent, by weight of the total amount of liquid mixed with the compact, is non-aqueous liquid.

The mixing of the water and the non-aqueous liquid with the carbonaceous compact can occur in one or several stages. The mixing can occur in one stage, wherein the carbonaceous compact is mixed with a mixture of water and a non-aqueous co-liquid. The mixing can, alternatively, occur in two or more stages. Thus, in one embodiment, the non-aqueous co-liquid is mixed with the carbonaceous compact, and thereafter the mixture of the co-liquid and the carbonaceous compact is mixed with water. Thus, in another embodiment, the water is mixed with the carbonaceous compact, and thereafter the mixture of the water and the carbonaceous compact is mixed with the non-aqueous co-liquid. Thus, in a third embodiment, part of the water and/or part of the non-aqueous liquid is mixed with the carbonaceous compact and thereafter the remainder of the water and/or the remainder of the non-aqueous co-liquid is mixed with the mixture of the carbonaceous compact and the liquid. Thus, in a fourth embodiment, the non-aqueous co-liquid is mixed with one portion of the carbonaceous material, and thereafter additional carbonaceous material and water is added to the mixture to form a slurry of the carbonaceous compact, water, and co-liquid; in this embodiment, the blending of various carbonaceous portions forms the carbonaceous compact in situ. Thus, in a fifth embodiment, the water is mixed with one portion of carbonaceous material, and thereafter additional carbonaceous material and non-aqueous co-liquid is added to the mixture to form a slurry of the carbonaceous compact, water, and co-liquid; in this embodiment, the blending of various carbonaceous fractions forms the carbonaceous compact in situ. Many other variations will suggest themselves to those skilled in the art; as long as, at some point in the process, carbonaceous material is mixed with water and non-aqueous co-liquid to form a slurry comprised of from about 60 to about 80 volume percent of the specified carbonaceous compact, from about 20 to about 40 volume percent of liquid (wherein at least about 90 weight percent of the liquid is water and from about 0.5 to about 10 weight percent of the liquid is non-aqueous co-liquid), then the process is within the scope of this invention.

The co-liquid used in the process of this invention is non-aqueous, that is, it is a fluid other than water. It is preferred that the co-liquid be an organic, non-aqueous liquid, although inorganic non-aqueous liquids also can be used.

Liquid alkanes containing from about 5 to about 17 carbon atoms can be used as the co-liquid in the process of this invention; the alkanes can be straight or

branched. By way of illustration and not limitation, some of the liquid alkanes which can be used in the process of this invention include, e.g., n-pentane, 2,2,4-trimethyl-pentane, n-hexane, n-octane, n-nonane, n-decane, n-undecane, n-dodecane, n-tridecane, n-tetradecane, n-pentadecane, n-hexadecane, n-heptadecane, and the like.

Liquid alkenes containing from about 6 to about 18 carbon atoms can be used as the co-liquid in the process of this invention. Thus, by way of illustration, one can use hexene-1, heptene-1, and octene-1 as the co-liquid in said process.

Liquid petroleum fuels, which are made by fractional distillation of petroleum, can be used as the co-liquid in the process of this invention. Thus, by way of illustration and not limitation, one can use one or more liquid fuels such as, e.g., number 1 fuel oil, number 2 fuel oil, number 4 fuel oil, number 5 fuel oil, and number 6 fuel oil; these fuel oils are described in A.S.T.M. Burner Fuel Specification D 396, the disclosure of which is hereby incorporated by reference into this specification. Thus, e.g., one can use petroleum liquids such as naphtha, high gas oil, low gas oil, catalytic cracked recycle oil, mixtures thereof, and other similar petroleum products.

Liquid vegetable oils can be used as the co-liquid in the process of this invention. Thus, e.g., one can use corn oil, bean oil, pine oil, etc. in said process.

Coal-tar liquid fuels can be used in the process of this invention; these fuels are made from the higher boiling fractions (over about 450° F.) of the crude tar produced by coke ovens and coal retorts at gas works. Thus, e.g., some of the coal-tar fuels which can be used in the process of this invention include, e.g., coal tar fuels (CTF's) 50, 100, 250, and 400.

Non-petroleum liquid fuels can be used as the co-liquid in the process of this invention. Thus, e.g., one can use oil shale, tar sands, and the like.

Liquid aromatic hydrocarbons which are derived from coal tar can be used as the co-liquid in the process of this invention. Thus, by way of illustration, one can use such aromatic hydrocarbons as benzene, toluene, ortho-xylene, meta-xylene, para-xylene, indene, and the like. Thus, e.g., one can use nitrogen liquid compounds derived from coal tar such as, e.g., pyridine, alpha-picoline, beta-picoline, gamma-picoline, quinoline, and the like. Thus, e.g., one can use oxygen-containing liquid compounds such as, e.g., ortho-cresol, meta-cresol, 2,4-dimethylphenol, and the like. Thus, e.g., one can use other liquid benzenoid hydrocarbons such as, e.g., hemimellitene, pseudocumene, isodurene, n-propylbenzene, cumene, n-butylbenzene, 1,3,5-triethylbenzene, styrene, allylbenzene, and the like.

Liquid monohydric alcohols containing from about 1 to about 18 carbon atoms can be used as the non-aqueous co-liquid in the process of this invention. Thus, by way of illustration and not limitation, one can use methyl alcohol, ethyl alcohol, n-propyl alcohol, isopropyl alcohol, allyl alcohol, n-butyl alcohol, isobutyl alcohol, tert-butyl alcohol, amyl alcohol, isoamyl alcohol, t-amyl alcohol, carbyl capryl alcohol, n-decyl alcohol, lauryl alcohol, benzyl alcohol, and the like can be used in the process of this invention.

Liquid polyhydric alcohols containing from about 2 to about 10 carbon atoms can be used in the process of this invention as the non-aqueous co-liquid. Thus, e.g., one can use ethylene glycol, 1,2-propanediol, 1,3-propanediol, 1,4-butanediol, 2,3-butanediol, 1,5-pen-

tanediol, glycerol, 1,2,4-butanetriol, 1,2,6-hexanetriol, and the like.

Lubricating oil can be used as the non-aqueous co-liquid in the process of this invention. In one embodiment, the lubricating oil contains from about 18 to about 26 weight percent of straight chain and possibly branched cahin paraffins, from about 43 to about 51 weight percent of alkylated naphthalanes containing 1, 2, or 3 rings, about 23 weight percent of alkylated naphthaene-  
10 aromatic hydrocarbons containing 2, 3, or 4 rings, and about 8 weight percent of asphaltic substances, which are considered to be largely aromatic. In another embodiment, the lubricating oil is "3-in-one household oil" which is sold by the Boyle-Midway Inc. of New York, N.Y. Other lubricating oils known to those skilled in the art can be used as the non-aqueous co-liquid in the process of this invention.

The invention contemplates the use of at least two distinct liquids (water and a non-aqueous co-liquid) which exist in different phases in the slurry. A slurry which contains only two phases (one solid phase and one liquid phase) is not within the scope of the present invention, which requires that the slurry contain at least one solid phase and at least two liquid phases.

In one of the preferred embodiments of the process of this invention, the carbonaceous compact is mixed with the water, the non-aqueous co-liquid, and from about 0.01 to about 4.0 weight percent of dispersing agent, based on the weight of dry carbonaceous solid material. It is preferred that the dispersing agent used be one (or more) which is most effective in reducing the viscosity of the slurry and dispersing the particles of carbonaceous material in the slurry. Means for determining the identity and the amount of the most effective dispersing agent for a given slurry will be described below for a coal-water mixture, it being understood that the technique described is applicable to other mixtures such as, e.g., coal-water-oil, coke-water-oil, graphite-water-oil, etc.

In general, for any given system, the identity of effective dispersing agents can be determined by measuring the effects of the dispersant upon the system at a given dispersant concentration; viscosity versus shear rate of the stirred coal-water slurry is measured while titrating with increasing amounts of the dispersing agent, and the point at which the slurry viscosity ceases to decrease is noted. For any given dispersant(s), and system, the most effective concentration is the one which gives the minimum viscosity under a given set of test conditions, and the efficiency of different dispersants can be compared by testing them with a given system under comparable concentration and test conditions. Thus, for example, one can grind a sample of coal in a laboratory size ball mill with porcelain or steel balls in water at 50 weight percent solids, e.g., for 24 hours or until all of the particles in the coal are less than 10 microns in size; other grinding devices known to those skilled in the art may also be used such as vibroenergy mills, stirred ball mills, or fluid energy mills. Small samples (about 500 milliliters apiece) of the system can then be deflocculated by adding various dispersing agents to the samples dry or preferably in solution dropwise, blending the mixture at any consistent blending energy (which may be gentle as mixing by hand, or at very high shear energy which will improve dispersion), and then measuring the viscosity at some constant shear rate by, e.g., using a Brookfield RVT viscometer at 100 revolutions per minute. The dispersing agent (or combination of dispersing agents)

which is found to produce the lowest viscosity for the system at a given shear rate and dispersing agent(s) concentration is the most effective for those conditions. This technique is described in detail in my U.S. Pat. No. 4,282,006, the disclosure of which is hereby incorporated herein by reference.

FIG. 2 illustrates one means of evaluating the effectiveness of surfactants for any given solid material. The curves of FIG. 2 represent data obtained using both a purported nonionic polymer CW-11 made by the Diamond Shamrock Process Chemicals Co. and an anionic lignosulfonate Polyfon-F made by Westvaco, Inc., adsorbed on an Australian coal. The fine coal ground to about 100% finer than 10 microns is slurried in distilled water at 0.01 weight percent solids. Aliquots are placed in test tubes, and increasing amounts of any candidate surfactant are added to each test tube. The test tube samples are thoroughly mixed and inserted into a sampler carousel. The Pen Kem System 3000 Electrophoretic Mobility Analyzer automatically and sequentially samples each test tube and measures the electrophoretic mobility of the coal particles and the specific conductance of the carrier liquid; pH can also be measured on each sample. In FIG. 2 the left ordinate gives the calculated zeta potential of the particles in millivolts, the right ordinate gives the specific conductance in micromhos of the carrier liquid. These variables are both measured as a function of the percent addition of each surfactant on a dry coal basis which is plotted on the abscissa. FIG. 2 shows that the purported nonionic CW-11 surfactant does have some anionic character. CW-11 has a zeta potential of -50 mv at 300% addition at 0.01% dry coal. Polyfon-F has a zeta potential of -55 mv at 200% addition on 0.01% dry coal. Furthermore, the specific conductance of the Polyfon-F at -55 m.v. zeta potential is greater than CW-11 at -50 m.v. These data establish Polyfon-F as a more chemically effective surfactant for use on this particular Australian coal.

The amount of dispersing agents which can be used will vary, depending upon such factors as the concentration of the coal in the slurry, the particle size and particle size distribution, the amount of ash minerals (i.e. clays and other minerals present), the temperature of the slurry, the pH, the original zeta potential of the particles, and the identity of the dispersing agent(s) and its concentration. In general, the dispersing agent preferably is present in the slurry, at from 0.01 to 4.0 weight percent based on the weight of dry coal. Procedurally, in determining the amount of a specific dispersing agent needed, a series of measurements can be made of viscosities versus shear rates versus zeta potential for a series of solids-liquid slurries containing a range of amounts of a particular dispersing agent for a constant amount of solids-liquid slurry. The data can be plotted and used as a guide to the optimum quantities of that agent to use to obtain near maximum or maximum zeta potential for that system. The coordinate of the chart at which the viscosity and/or zeta potential is not changed significantly by adding more agent is selected as an indication of the optimum quantity at maximum zeta potential, and the amount is read from the base line of the chart. The viscosity and amount read from the titration chart is then compared with an equivalent chart showing a correlation between viscosity, amount, and maximum zeta potential. An amount of electrolyte and/or dispersing agent(s) required to provide a maximum or near

maximum zeta potential and a selected viscosity can then be used to make a solids-liquid slurry.

Any dispersing agent which disperses the carbonaceous particles in the water can be used. As is known to those skilled in the art, the dispersing agent can be inorganic. Thus, for example, sodium hydroxide can be used with some carbonaceous materials. The dispersing agent can be, and preferably is, organic, i.e., it contains carbon. The dispersing agent is preferably an anionic organic surfactant.

It is preferred that the dispersing agent used be an organic compound which encompasses in the same molecule two dissimilar structural groups, e.g., a water soluble moiety, and a water insoluble moiety. It is preferred that said dispersing agent be a surfactant. The term "surface-active agent", or "surfactant", as used herein indicates any substance that alters energy relationships at interfaces, and, in particular, a synthetic or natural organic compound displaying surface activity including wetting agents, detergents, penetrants, spreaders, dispersing agents, foaming agents, etc.

The surfactant used is preferably an organic surfactant selected from the group consisting of anionic surfactants, nonionic surfactants, cationic surfactants, and amphoteric surfactants. It is preferred that the surfactant be either anionic or cationic. In the most preferred embodiment, the surfactant is anionic.

It is preferred that the molecular weight of the surfactant used be at least about 200. As used herein, the term "molecular weight" refers to the sum of the atomic weights of all the atoms in a molecule.

In one preferred embodiment, the surfactant is anionic and its solubilizing group(s) is selected from the group consisting of a carboxylate group, a sulfonate group, a sulfate group, a phosphate group, and mixtures thereof. By way of illustration, one of these preferred anionic surfactants is a polyacrylate having the general formula.



wherein  $n$  is a whole number of at least 3 and  $M$  is selected from the group consisting of hydrogen, sodium, potassium, and ammonium.

In another preferred embodiment, the surfactant is cationic and its solubilizing group(s) is selected from the group consisting of a primary amine group, a secondary amine group, a tertiary amine group, a quaternary ammonium group and mixtures thereof.

In yet another embodiment, the surfactant is amphoteric. In this embodiment, the surfactant has at least one solubilizing group selected from the group consisting of a carboxylate group, a sulfonate group, a sulfate group, a phosphate group, and mixtures thereof; and the surfactant also has at least one solubilizing group selected from the group consisting of a primary amine group, a secondary amine group, a tertiary amine group, a quaternary ammonium group, and mixtures thereof.

In one of the more preferred embodiments, the surfactant used is comprised of at least about 85 weight percent of a structural unit of the formula:

5



10 wherein  $R_1$  and  $R_2$  are independently selected from the group consisting of alkyl of from about 1 to about 6 carbon atoms and hydrogen;  $a$ ,  $b$ ,  $c$ , and  $d$  are integers independently selected from the group consisting of 0, 1, 2, 3, 4, 5, 6, 7, and 8, and  $X_2$  and  $X_3$  are independently selected from the group consisting of a carboxylate group, a sulfonate group, a sulfate group, a phosphate group, a nitro group, a halo group selected from the group consisting of chloro, bromo, fluoro, and iodo,  $-\text{CN}$ , an alkoxy group containing from 1 to about 6 carbon atoms, and a group of the formula  $-\text{R}_3\text{OR}_4$  wherein  $R_3$  and  $R_4$  are an alkyl containing from about 1 to about 3 carbon atoms. The starting materials which can be used to prepare these surfactants are well known to those skilled in the art and include, e.g., naphthalene- $\alpha$  sulfonic acid (dihydrate), naphthalene- $\beta$ -sulfonic acid (monohydrate),  $\alpha$ -nitronaphthalene,  $\beta$ -nitronaphthalene,  $\alpha$ -naphthylamine,  $\beta$ -naphthylamine,  $\alpha$ -naphthol,  $\beta$ -naphthol,  $\alpha$ -naphthoic acid,  $\beta$ -naphthoic acid,  $\alpha$ -chloronaphthalene,  $\alpha$ -bromonaphthalene,  $\beta$ -bromonaphthalene,  $\beta$ -chloronaphthalene,  $\alpha$ -naphthomitrile,  $\beta$ -naphthonitrile, 1,5-dinitronaphthalene, 1,8-dinitronaphthalene,  $\beta$ -methylnaphthalene, 1-nitro-2-methylnaphthalene, 2-methylnaphthalene-6-sulfonic acid, 2,6-dimethylnaphthalene,  $\beta$ -6-methylnaphtholpropionic acid, 1,6-dibromo-2-naphthol, 6-bromo-2-naphthol, 1,6-dibromonaphthalene, 6-bromo-2-naphthol, and the like. Again, it is preferred that at least one of the atoms in this surfactant be an alkali metal selected from the group consisting of sodium, potassium, ammonium, and mixtures thereof. One of the most preferred surfactants from this group is the alkali metal salt of a condensed mononaphthalene sulfonic acid. This acid, whose preparation is described in U.S. Pat. No. 3,067,243 (the disclosure of which is hereby incorporated by reference into this specification), can be prepared by sulfonating naphthalene with sulfuric acid, condensing the sulfonated naphthalene with formaldehyde, and then neutralizing the condensate so obtained with sodium hydroxide. This alkali or  $\text{NH}_4^+$  metal salt of a condensed mono naphthalene sulfonic acid is comprised of at least about 85 weight percent of a repeating structural unit of the formula

25

30

35

40

45

50

55



wherein  $M$  is an alkali metal selected from the group consisting of sodium, potassium, and ammonium and  $a$  is an integer of from 1 to 8. Comparable compounds with a benzene rather than naphthalene nucleus also can be used.

Examples of anionic organic surfactants which have been found particularly advantageous are also described

below. In some cases, mixtures of two or more of these surfactants beneficially can be used.

Some of the surfactants sold by the Diamond Shamrock Chemical Company of Morristown, N.J. can be used in this invention. Thus, by way of example, one can use surfactants such as Lomar D (the sodium salt of a condensed mono naphthalene sulfonic acid), Lomar PW (sodium neutralized naphthalene sulfonic acid), Lomar PWA (ammonia salt of a condensed mono naphthalene sulfonic acid), A23, Nopcosperse VFG (condensed alkyl naphthalene sulfonate), and Nopcosperse VEO (polymerized alkyl naphthalene sulfonate).

Some of the surfactants sold by the R. T. Vanderbilt Company of Norwalk, Conn. can be used in this invention. Thus, by way of example, one can use Darvan #1 (sodium naphthalene sulfonic acid formaldehyde), Darvan #2 (sodium salts of polymerized substituted benzoid alkyl sulfonic acids), and Darvan #6 (sodium salts of polymerized alkyl naphthalene sulfonic acid).

Some of the surfactants sold by the Westvaco-Poly-  
chemicals, Charleston Heights, S.C. can be used in this  
invention. Thus, for example, one can use Reax 88B  
(sodium salt of a chemically modified low molecular  
weight kraft lignin polymer solubilized by 4 sulfonate  
groups), Reax 15B (sodium salt of sulfonated modified  
kraft lignin), Reax 100M (reaction product of selected  
modified kraft lignins with a high sulfonic acid group  
content), and Polyfon 0 (sugar-free, sodium-based sulfo-  
nates of Kraft lignin).

Some of the surfactants sold by the W R Grace & 30 Co., Organic Chemicals Div., Lexington, Maine can be used in this invention. Thus, by way of illustration, one can use Daxad 11, 11G, 15, or 19 (sodium salts of polymerized alkyl naphthalene sulfonic acids), Daxad 30 or 31 (sodium salt of a carboxylated polyelectrolyte), or 35 Daxad 32 (ammonium salt of a carboxylated polyelectrolyte).

Some of the surfactants sold by the Rohm & Haas Company of Philadelphia, Pa. can be used in this invention. Thus, for example, one can use, Triton X-100 (octylphenoxy polyethoxy ethanol), Triton N-101 (nonylphenoxy polyethoxy ethanol), Tamol 731 (sodium salt of polymeric carboxylic acid), Tamol 850 (sodium salt of polymeric carboxylic acid), and Tamol SN (sodium salt of condensed naphthalene sulfonic acid).

Some of the surfactants produced by the Hamblet & Hayes Co. of Salem, Mass. can be used in this invention. Thus, e.g., one can use Tek Tan ND (condensed naphthalene sulfonate).

Some of the surfactants made by the National Starch and Chemical Corp. of Bridgewater, N.J. can be used in this invention. Thus, one can use Versa TL 70 (an anionic polyelectrolyte of sodium polystyrene).

Some of the surfactants made by the Thompson-Hayward Chemical Co. of Kansas City, Kans. also can be used in this invention. Thus, for example, one can use T-DET N-100 (nonylphenol-100 mole ethylene oxide adduct), T-DET N-50 (nonylphenol-50 mole ethylene oxide adduct), T-DET N-14 (nonylphenol-14 mole ethylene oxide adduct), T-DET N-9.5 (nonylphenol-9.5 mole ethylene oxide adduct), T-DET C-40 (polyethoxylated castor oil with 40 moles of ethylene oxide), and the like.

Renex 30, a polyoxyethylene (12) tridecyl ether manufactured by the ICI Corp. of Wilmington, Del., also 65 can be used in this invention.

Some of the Duponol surfactants manufactured by the E. I. duPont De Nemours & Co. of Wilmington,

Del. also can be used in this invention. Thus, one can use Dupanol WA and Dupanol WAQ (both sodium lauryl sulfate).

Some of the surfactants made by the Scher Chemicals, Inc. of Clifton, N.J. also can be used in this invention. Thus, one can use cocamidopropyl betaine.

One class of surfactants which can beneficially be used in this invention are the polyalkyleneoxide non-ionic surfactants having a hydrophobic portion and a hydrophilic portion, wherein the hydrophilic portion comprises at least about 100 units of ethylene oxide. These surfactants are disclosed in U.S. Pat. No. 4,358,293, the disclosure of which patent is hereby incorporated by reference into this specification.

The polyalkyleneoxide nonionic surfactants suitable for use in the invention include the glycol ethers of alkylated phenols having a molecular weight of at least about 4,000 of the general formula:



wherein R is substituted or unsubstituted alkyl of from 1 to 18 carbon atoms, preferably 9 carbon atoms; substituted or unsubstituted aryl, or an amino group, and n is an integer of at least about 100. The substituents of the alkyl and aryl radicals can include halogen, hydroxy, and the like.

Other suitable nonionic surfactants are the poly(oxyethylene)poly(oxypropylene)-poly(oxyethylene) or as otherwise described propoxylated, ethoxylated propylene glycol nonionic surfactant block polymers having a molecular weight of at least about 6,000 of the general formula:



wherein  $a$ ,  $b$  and  $c$  are whole integers and wherein  $a$  and  $c$  total at least about 100.

Still other polyalkyleneoxide nonionic surfactants suitable for use in the invention are the block polymers of ethylene and propylene oxide derived from nitrogen-containing compositions such as ethylene diamine and having a molecular weight of at least about 14,000 of the general formula:



wherein R<sub>1</sub> is an alkylene radical having 2 to 5 carbon atoms preferably 2; R<sub>2</sub> is alkylene radical having 3 to 5 carbon atoms, preferably 3; a, b, c, d, e, f, g and h are whole integers; and e, f, g and h total at least about 100.

One of the preferred surfactants is



wherein M is alkali metal (and most preferably is sodium) and n is less than 200 and, preferably, less than 100.

While, in one embodiment, the use of the sodium, potassium, or ammonium salts of condensed mononaphthalene sulfonic acid is preferred, it is to be understood that the condensed mononaphthalene sulfonic acid can be used with the addition of sodium, potassium, or ammonium alkali to form the corresponding alkali metal salt of that acid in situ.

Yet another of the surfactants which can be used in this invention is an anionic, alkylaryl sulfonate which is liquid and has an HLB number of from about 8.0 to about 15.0.

Yet another preferred surfactant is a lignin-based dispersing agent which is water soluble and which contains a sulfite lignin which ranges in molecular weight from about 1,000 to about 50,000 and whose basic lignin unit is a substituted phenylpropane. This lignin can be generated by the acid sulfite wood pulping process.

Yet another preferred surfactant is a lignin-based dispersing agent which is water-soluble and which contains an alkali lignin isolated from sulfate pulping black liquor generated in the alkalin sulfate wood pulping process.

Yet another class of preferred surfactant is a complex polymerized organic salt of sulfonic acids of the alkylaryl type such as, e.g., sodium naphthalene sulfonic acid formaldehyde, sodium salts of polymerized alkyl naphthalene sulfonic acid, and the like.

Another preferred class of surfactants is the lignosulfonates. These lignosulfonates have an equivalent weight of from about 100 to about 350, contain from about 2 to about 60 phenyl propane units (and, preferably, from about 3 to 50 phenyl propane units), and are made up of cross-linked polyaromatic chains. Some of the preferred lignosulfonates include those listed on page 293 of McCutcheon's "Emulsifiers and Detergents", North American Edition (McCutcheon Division, MC Publishing Co., Glen Rock, N.J., 1981) and in the other portions of McCutcheon's which describes said lignosulfonates, the disclosure of which is hereby incorporated by reference into this specification. In one preferred embodiment, the lignosulfonate surfactant contains from about 0.5 to about 8.0 sulfonate groups. In this preferred embodiment, one species has 0.5 sulfonate groups, one has one sulfonate group, one has two sulfonate groups, and one has four sulfonate groups, and one has 7.5 sulfonate groups.

Applicant does not wish to be bound to any particular theory. However, he believes that a dispersing agent in a aqueous slurry system might perform at least three functions. In the first place, it is believed that a water soluble dispersing agent, which also serves as a wetting agent (such as an organic surfactant), functions to promote the wettability of the carbonaceous particles by water. As used herein, the term "wetting" indicates covering or penetrating the carbonaceous particle surface with a bound water layer. Such a wetting agent might or might not be needed, depending upon the surface chemistry of the particle, its hydrophobicity and the associated electrochemistry of its inherent bound water layers. For example, inherent bed moisture, oxidation state of the particle, and chemical compounds already present in natural carbonaceous deposits may allow wetting of the ground material by added water.

In the second place, a dispersing agent might function to promote deflocculation of carbonaceous particles,

preferably in the presence of advantageous electrolytes. As used herein, the term "deflocculating" indicates dispersion of particles, preferably of colloidal sized carbonaceous particles. Thus, e.g., a "deflocculating agent" includes a dispersing agent which promotes formation of a colloidal dispersion of colloidal sized particles in a solids-liquid slurry. It has been found that the presence of large, monovalent cations—such as  $\text{Na}^+$ ,  $\text{Li}^+$ , or  $\text{K}^+$ —tend to promote deflocculation of 5 colloidal sized carbonaceous particles in a solids-liquid slurry. However, higher valence cations—such as  $\text{Ca}^{+2}$ ,  $\text{Al}^{+3}$ , and  $\text{Mg}^{+2}$ —tend to cause said particles to flocculate under certain conditions. Consequently, an organic anionic surfactant which wets the carbonaceous 10 particles and contains a residual  $\text{Na}^+$  and/or  $\text{K}^+$  and an  $\text{Li}^+$  can be a very effective deflocculant for the slurry.

In the third place, in some cases the dispersing agent enhances the pumpability of the system. It is believed that this effect occurs because of enhancement or inhibition 15 of the bound, or semi-rigid, water layer because the dispersing agent provides a cation as a counterion for the bound water layer, thereby affecting the yield pseudoplastic index (slope of a plot of log viscosity versus log shear rate) of the mass. Preferably, the cation provided by the dispersing agent is  $\text{NH}_4^+$ ,  $\text{Na}^+$  and/or  $\text{K}^+$ . Consequently, it is preferred to incorporate an 20 advantageous electrolyte, such as an ammonium or alkali metal base, into an aqueous slurry to increase deflocculation of the slurry and thus improve its yield 25 pseudoplasticity.

It is preferred that the dispersing agent(s) used in the system provide one or more ions to the system. As used in this specification, the term "ion" includes an electrically charged atom, an electrically charged radical, or an electrically charged molecule.

In one preferred embodiment, the dispersing agent(s) used in the system provides one or more counterions which are of opposite charge to that of the surface of the carbonaceous particles. The charge on the surface of the carbonaceous particles in water is generally negative, and thus it is preferred that said counterions have a positive charge. The most preferred positively charged ions are the sodium and potassium cations and the ammonium radical.

In one embodiment it is preferred that the dispersing agent(s) used in the system be a polyelectrolyte which, preferably, is organic. As used in this specification, the term "polyelectrolyte" indicates a polymer which can be changed into a molecule with a number of electrical 40 charges along its length. It is preferred that the polyelectrolyte have at least one site on each recurring structural unit which, when the polyelectrolyte is in aqueous solution, provides electrical charge; and it is more preferred that the polyelectrolyte have at least two such sites per recurring structural unit. In a preferred embodiment, said sites comprise ionizable groups selected from the group consisting of ionizable carboxylate, sulfonate sulfate, and phosphate groups. Suitable polyelectrolytes include, e.g., the alkali metal and ammonium 45 salts of polycarboxylic acids such as, for instance, polyacrylic acid; the sodium salt of condensed naphthalene sulfonic acid; polyacrylamide; and the like.

In one preferred embodiment, the slurry system contains from about 0.05 to about 4.0 weight percent by 50 weight of dry solids in the slurry, of an electrolyte which, preferably, is inorganic. As used in this specification, the term "electrolyte" refers to a substance that dissociates into two or more ions to some extent in

water or other polar solvent. This substance can be, e.g., an acid, base or salt.

In a more preferred embodiment, the slurry system is comprised of from about 0.05 to about 2.0 weight percent of an inorganic electrolyte. In the most preferred embodiment, said system is comprised of from about 0.1 to about 0.8 weight percent of said electrolyte. In the most preferred embodiment, the system contains from about 0.1 to about 0.5 percent of inorganic electrolyte.

Any of the inorganic electrolytes known to those skilled in the art can be used in the coal-water system. Thus, by way of illustration and not limitation, one can use the ammonia or alkali metal salt of hexametaphosphates, pyrophosphates, sulfates, carbonates, hydroxides, and halides. Alkaline earth metal hydroxides can be used. Other inorganic electrolytes known to those skilled in the art also can be used.

In one preferred embodiment, the inorganic electrolyte is of the formula



wherein M is an alkali metal selected from the group consisting of lithium, sodium, potassium, rubidium, cesium, and francium; b is the valence of metal M; a is the valence of anion Z; and Z is an anion selected from the group consisting of hexametaphosphate, pyrophosphate, silicate, sulfate, carbonate, hydroxide, and halide anions. It is preferred that Z be selected from the group consisting of carbonate, hydroxide, and silicate anions. The most preferred electrolytes are selected from the group consisting of potassium carbonate, sodium hydroxide, and  $Na_2SiO_3 \cdot 9H_2O$ .

It is preferred that the slurry system contain both said dispersing agent(s) and said inorganic electrolyte(s) and that from about 0.05 to about 10.0 parts (by weight) of the inorganic electrolyte are present for each part (by weight) of the dispersing agent(s) in the system.

It is preferred that the total concentration of both the dispersing agent(s) and/or the inorganic electrolyte be from 0.05 to 4.0 weight percent.

In one preferred embodiment, the grinding mixture is comprised of dispersing agent(s) and inorganic electrolyte agent(s) which, when dissolved in water, provide electrically charged ions to the mixture. The amount of electrically charged ions preferably present in the mixture ranges from about 0.01 to about 2.5 weight percent, based upon weight of dry carbonaceous materials and most preferably is from about 0.05 to about 2.0 weight percent. Said concentration of electrically charged ions can be calculated by first calculating the weights of the ions in each of the dispersing agent(s) and the electrolyte agent(s), adding said weight(s), and then dividing the total ion weight by the weight of the dry coal.

By way of illustration, in one embodiment 0.75 grams of sodium hydroxide and 0.75 grams of sodium decyl benzene sulfonate were added to a mixture comprised of 100 grams of dry coal. The weight of the sodium ion provided by the caustic was equal to  $22/40 \times 0.75$  grams; and it equals 0.4125 grams. The weight of the sodium ion provided by the sodium decyl benzene sulfonate was equal to  $22/294 \times 0.75$  grams; and it equals 0.0561 grams. The total weight of the sodium ion provided by both the caustic electrolyte and the sulfonate dispersing agent was 0.4686 grams. Thus, the slurry contained 0.468 weight percent of sodium ion.

In one of the preferred embodiments of the process of this invention, a slurry is prepared from a specified grinding mixture which contains from about 60 to about

82 parts by volume of carbonaceous material, from about 18 to about 40 parts by volume of carrier liquid, and from about 0.01 to about 4.0 parts, by weight of dry carbonaceous material, of dispersing agent; the pH of this grinding mixture is from about 5 to about 12. The carrier liquid in the grinding mixture contains both water and non-aqueous co-liquid, at least about 90 weight percent of the liquid being water and from about 0.05 to about 10 weight percent of the liquid being non-aqueous co-liquid.

The grinding mixture can be provided either prior to or during grinding. In one embodiment, the carbonaceous material, carrier liquid, and dispersant are mixed to provide the grinding mixture, and the mixture so provided is then ground to produce a stable slurry. The aforementioned materials can be mixed by means well known to those skilled in the art including, e.g., blending them together, grinding them together, and combinations of blending and grinding them together. In another embodiment, all of the carbonaceous material desired in the grinding mixture is mixed with less than all of the carrier liquid and/or dispersant desired in the grinding mixture, and the incomplete mixture is then ground while the remainder of the carrier liquid and/or the dispersant is added during grinding; in this embodiment, the desired grinding mixture is generated in situ during grinding. In another embodiment, less than all of the carbonaceous material desired in the grinding mixture is mixed with carrier liquid and dispersant, and the incomplete mixture is then ground while the remainder of the carbonaceous material is added during grinding; in this embodiment, the desired grinding mixture is also generated in situ during grinding. Other embodiments will be apparent to those skilled in the art.

In one preferred embodiment of this invention, at least two consists of carbonaceous material are mixed with carrier fluid to prepare the grinding mixture. Both of said consists of carbonaceous material can be produced by wet grinding; thus, e.g., one of the consists can be produced by grinding coal at a high solids content (60-82 volume percent) in the presence of water and optionally, surfactant, the second of the consists can be produced by grinding coal at a lower solids content (30-60 volume percent) in a ball mill or a stirred ball mill, and the first and the second coal consists can be ground together with each other (and, optionally, with one or more additional consists produced by wet and/or dry grinding) at a solids content of from about 60 to about 82 volume percent in the optional presence of from about 0.01 to about 4.0 weight percent of dispersant and water. Alternatively, both of said consists of carbonaceous material can be produced by dry grinding; thus, e.g., one of the consists can be prepared by grinding one pulverized coal (i.e., coal which has been milled or ground to a consist of about 20 mesh by 0) in, e.g., a ring roller mill, a second or more of the consists can be prepared by dry grinding a second pulverized coal in, e.g., a micronizer fluid energy (jet) mill, and the two ground dry fractions are then blended in a blending tank at a solids concentration of from 60-90 volume percent with water and, optionally, 0.01 to 4.0 weight percent of dispersant at a high shear stress in a mixer such as a Greerco in-line mixer.

Alternatively, at least one of said consists can be produced by wet grinding, and at least one of said consists can be produced by dry grinding; thus, e.g., one of the consists can be produced by wet grinding coal at a

low solids content (30-60 volume percent) in the presence of water and, optionally, dispersant, a second of the consists can be produced by dry grinding pulverized coal in either a micronizer fluid energy (jet) mill, or a ring roller mill, and the consists produced by wet and dry grinding are then blended in a blending tank at a solids concentration of 60-82 volume percent water and, optionally, 0.01 to 4.0 weight percent of dispersant at a high shear stress in a mixer such as a Greerco in-line mixer.

Alternatively, one can prepare the grinding mixture by wet grinding (or regrinding) slurry comprised of carbonaceous material to produce the fine consist for the mixture. Thus, by way of illustration, a fine consist can be prepared by regrinding a "final slurry" product at a concentration of from about 40 to about 60 weight percent solids (and preferably at from about 45 to about 55 weight percent of solids) in, e.g., a stirred ball mill until the median particle size of the slurry is from about 4 to about 20 microns. The coarse consist can be produced by dry crushing (in, e.g., a roll crusher, a gyratory crusher, a cage mill, etc.) the carbonaceous material to a nominal  $\frac{3}{8}'' \times 0$  size so that the median particle size of the coarse fraction exceeds 40 microns. The coarse and fine fractions can then be combined with each other, carrier liquid, and dispersing agent to produce a grinding mixture comprised of from about 60 to about 82 volume percent of carbonaceous material, from about 18 to about 40 volume percent of carrier liquid, and from about 0.01 to about 4.0 weight percent of dispersion dispersing agent.

The fine consist in this particular embodiment can alternatively be made by regrinding a dry pulverized coal at a concentration of from about 40 to about 60 weight percent solids until the median particle size of the fine consist is from about 4 to about 20 microns.

The aforementioned processes are all illustrated in FIG. 1.

It will be apparent to those skilled in the art that there are many other arrangements wherein two consists of carbonaceous material can be mixed with carrier liquid to produce the grinding mixture; they are intended to be within the scope of the invention.

The solid carbonaceous material in the preferred grinding mixture consists essentially of at least one fine solid carbonaceous material and at least one coarse solid carbonaceous material. From about 2 to about 50 weight percent of the solid carbonaceous material in the grinding mixture can be comprised of fine solid carbonaceous material with a median particle size of from about 0.5 to about 40 microns; it is preferred that from about 4 to about 40 weight percent of the solid carbonaceous material in the grinding mixture be comprised of fine solid carbonaceous material with a median particle size of from about 1 to about 30 microns; and it is even more preferred that from about 6 to about 30 weight percent of the solid carbonaceous material in the grinding mixture be comprised of fine solid carbonaceous material with a median particle size of from about 2 to about 20 microns. From about 50 to about 98 weight percent of the solid carbonaceous material in the grinding mixture can be comprised of coarse solid carbonaceous material with a median particle size greater than 40 microns.

The preferred grinding mixture can contain one fine carbonaceous solid fraction or several fine carbonaceous solid fractions, which may be the same or different carbonaceous materials; regardless of whether one

or several such fine fractions are present in this grinding mixture, from about 2 to about 50 weight percent of the solid carbonaceous material in this grinding mixture has a median particle size of from about 0.5 to about 40 microns.

The preferred grinding mixture can contain one coarse carbonaceous solid fraction or several coarse carbonaceous solid fractions, which may be the same or different carbonaceous materials; regardless of whether one or several such coarse fractions are present in this grinding mixture, from about 50 to about 98 weight percent of the solid carbonaceous material in this grinding mixture has a median particle size greater than about 40 microns. It is preferred that the grinding mixture be comprised of from about 60 to about 96 weight percent of said coarse solid carbonaceous material, and it is more preferred that said grinding mixture be comprised of from about 70 to about 94 weight percent of said coarse solid carbonaceous material.

The grinding mixture can be comprised of discrete fine fraction(s) and coarse fraction(s) of solid carbonaceous material. Alternatively, the grinding mixture can be comprised of a single fraction of carbonaceous material, which was produced by mixing said coarse fraction(s) and said fine fraction(s). As long as a particle size analysis of the solid carbonaceous material in the preferred grinding mixture reveals that from about 2 to about 50 weight percent of said material has a median particle size of from about 0.5 to about 40 microns, and that from about 50 to about 98 weight percent of said material has a median particle size greater than 40 microns, then the consists of carbonaceous material are suitable for use in the preferred grinding mixture of this invention. The particle size analysis of the carbonaceous material will show substantial undulation at one or more points in the entire CPFT plot where two or more size distributions have obviously merged.

The carbonaceous solid is preferably mixed with from about 0.01 to about 4.0 weight percent (based upon dry weight of carbonaceous solid) of dispersing agent to produce said grinding mixture. In the case where at least two consists of carbonaceous solid material are mixed with liquid, (1) both of the consists can be dry ground and mixed with liquid and dispersant, (2) the dispersant can be mixed with the liquid, and the dry ground consists can be mixed with the liquid-dispersant mixture; (3) one of the consists can be dry ground, a second of the consists can be wet ground with part or all of the dispersant, and the ground consists can be mixed with the balance of the liquid and dispersant which was not theretofore mixed with the consists, or (4) some or all of the dispersant can be wet ground with one or both of the consists, and the ground consists can then be mixed with the liquid and the balance of the dispersant which was not theretofore mixed with the consists; (5) one or more consists can be wet ground with no dispersant and insufficient total water and then blended with dispersant and the balance of the water and/or other consist blends.

The grinding mixture used preferably contains from about 60 to about 82 volume percent of one or more carbonaceous solid materials. It is preferred that said grinding mixture contain from about 64 to about 81 volume percent of said carbonaceous solid material. In a more preferred embodiment, the grinding mixture contains from about 75 to about 80 volume percent of said solid carbonaceous material.

The grinding mixture used generally has a pH of from about 5 to about 12. It is preferred that the pH of the grinding mixture be from about 7 to about 11.

The grinding mixture can be produced by means well known to those skilled in the art. One such means will be described below, it being understood that other comparable means can be used.

In one process, the grinding mixture is prepared by a process comprising the steps of (1) preparing a slurry without fines which slurry contains from about 40 to about 60 weight percent of solid carbonaceous material; (2) grinding said slurry to a fine grind until the median particle size of the carbonaceous particles in the slurry is from about 0.5 to about 40 microns; (3) crushing dry coal until at least 98 weight percent of its particles are smaller than 50 mesh (300 microns), provided that the median particle size of the crushed coal exceeds about 40 microns; and (4) blending the ground slurry and the crushed coal in specified proportions, together with dispersant.

In the first step of this process, a carbonaceous slurry comprised of from about 40 to about 70 volume percent of carbonaceous solid material and from about 60 to about 30 volume percent of carrier liquid is prepared; it is preferred that the slurry contain from about 35 to about 65 volume percent of carbonaceous solid material and from about 65 to about 35 volume percent of carrier liquid. The slurry can be produced by grinding a mixture containing from about 40 to about 70 volume percent of solid carbonaceous material and from about 70 to about 40 volume percent of carrier liquid.

In the second step of this process, the slurry from step one of the process is fine ground in a fine grinder until the median particle size of its particles of solid carbonaceous material is from about 0.5 to about 40 microns and, preferably, from about 1 to about 30 microns. It is most preferred to fine grind the slurry until the median particle size of its particles of solid carbonaceous material is from about 2 to about 20 microns. The slurry can be fine ground by means well known to those skilled in the art. Thus, by way of example, the slurry can be fine ground in a stirred ball mill, a colloid mill, a vibratory mill, etc.

In the third step of this process, dry carbonaceous material is separately ground until its median particle size is greater than about 40 microns and about 98 percent of its particles are smaller than  $\frac{3}{8}$  inch. One may start with any size dry coal in this step and grind it.

In the fourth step of this process, the fine and coarse carbonaceous fractions are mixed until a grinding mixture with the desired composition is obtained.

As indicated above, the aforementioned grinding mixture can be provided by mixing solid carbonaceous material, carrier liquid, and dispersing agent. Thereafter, the grinding mixture can be wet ground until a slurry with specified properties is produced. Thus, in general, the grinding can be continued to produce a stable, solids-liquid slurry comprising a consist of finely-divided particles of solid carbonaceous material dispersed in said liquid, wherein:

(a) said slurry is comprised of at least about 60 volume percent of said solid carbonaceous material (dry basis), less than about 40 volume percent of said liquid, and from about 0.01 to about 4.0 weight percent (based on weight of dry solid carbonaceous material) of dispersing agent;

(b) said slurry has a yield stress of from about 3 to about 18 Pascals and a Brookfield viscosity at a solids

content of 70 volume percent, ambient temperature, ambient pressure, and a shear rate of 100 revolutions per minute of less than 5,000 centipoise;

(c) said consist has a specific surface area of from about 0.8 to about 4.0 square meters per cubic centimeter and an interstitial porosity of less than 20 volume percent;

(d) from about 5 to about 70 volume percent of said particles of solid carbonaceous material are of colloidal size, being smaller than about 3 microns;

(e) said consist of finely-divided particles of solid carbonaceous material has a particular size distribution substantially in accordance with the following formula:

$$\frac{CPFT}{100} = \sum_{j=1}^k \left[ X_j \left( \frac{D_{sj}^{Nj} - D_{sj}^{Nj}}{D_{Lj}^{Nj} - D_{sj}^{Nj}} \right) \right]$$

$$\text{where } \sum_{j=1}^k X_j = 1.0$$

$$\text{and where if } D < D_{sj} \left( \frac{D_{sj}^{Nj} - D_{sj}^{Nj}}{D_{Lj}^{Nj} - D_{sj}^{Nj}} \right) = 0.0$$

$$\text{and where if } D > D_{Lj} \left( \frac{D_{sj}^{Nj} - D_{sj}^{Nj}}{D_{Lj}^{Nj} - D_{sj}^{Nj}} \right) = 1.0$$

35 wherein:

1. CPFT is the cumulative percent of said solid carbonaceous material finer than a certain specified particle size D, in volume percent;

2. k is the number of component distributions in the consist and is at least 1;

3. X<sub>j</sub> is the fractional amount of the component j in the consist, is less than or equal to 1.0, and the sum of all of the X<sub>j</sub>'s in the consist is 1.0;

4. n is the distribution modulus of fraction j and is greater than about 0.001;

5. D is the diameter of any particle in the consist and ranges from about 0.05 to about 1180 microns;

6. D<sub>s</sub> is the diameter of the particle in fraction j, measured at 1% CPFT on a plot of CPFT versus size D, is less than D<sub>Lj</sub> and is greater than 0.05 microns;

7. D<sub>Lj</sub> is the diameter of the size modulus in fraction j, measured by sieve size or its equivalent, and is from about 10 to about 1180 microns;

(f) the net zeta potential of said colloidal size particles of solid carbonaceous material is from about 15 to about 85 millivolts; and

(g) the concentration of solid carbonaceous material in said slurry, the interstitial porosity of said consist, the specific surface area of said consist, and the zeta potential of said colloidal size particles of solid carbonaceous material are interrelated in accordance with the following formula:

$$V_s + P_s + SA + 240/ZP = H$$

wherein:

1. V<sub>s</sub> is the percent, by volume, of solid carbonaceous material in said slurry;

2. P is the porosity of said consist in the slurry, in percent;
3. S.A. is the specific surface area of said consist in said slurry, in square meters per cubic centimeter;
4. Z.P. is the net zeta potential of said colloidal size 5 particles of carbonaceous material in said consist, in millivolts, and
5. H is from about 75 to about 98.

The slurry produced by the grinding process has a yield stress of from about 3 to about 18 Pascals. It is 10 preferred that the yield stress be from about 5 to about 15 Pascals, and it is more preferred that the yield stress be from about 7 to about 12 Pascals. As is known to those skilled in the art, the yield stress is the stress which must be exceeded before flow starts. A shear stress versus shear rate diagram for a yield pseudoplastic or a Bingham plastic fluid usually shows a non-linear hump in the rheogram at the onset of flow; extrapolating the relatively linear portion of the curve back to the intercept of the shear stress axis gives the yield stress. See, for example, W. L. Wilkinson's "Non-Newtonian Fluids, Fluid Mechanics, Mixing and Heat Transfer" (Pergamon Press, New York 1960), pages 1-9, the disclosure of which is hereby incorporated herein by reference. Also see Richard W. Hanks, et al's "Slurry Pipeline Hydraulics and Design" (Pipeline Systems Incorporated, Orinda, Calif., 1980), pages II-1 to II-10, the disclosure of which is also hereby incorporated herein by reference.

The Brookfield viscosity of the slurry is less than 30 about 5,000 centipoise. The Brookfield viscosity is tested after the solids concentration of the slurry is adjusted to a solids content of 70 volume percent (the slurry is either diluted or concentrated until it has this concentration of solids) at ambient temperature, ambient pressure, and a shear rate of 100 revolutions per minute. It is preferred that the viscosity of the slurry be less than 4,000 centipoise. It is more preferred that the viscosity of the slurry be less than 3,000 centipoise. In an even more preferred embodiment, the viscosity of the slurry is less than 2,000 centipoise. In the most preferred embodiment, the viscosity of the slurry is less than 1,000 centipoise.

The term "Brookfield viscosity", as used in this specification, describes viscosity as measured by conventional techniques by means of a Brookfield Synchro-Lectric Viscosimeter (manufactured by the Brookfield Engineering Laboratories, Stoughton, Mass., U.S.A.).

The solids-liquid slurry produced contains a consist of finely divided particles of solid carbonaceous material dispersed in said liquid. Said consist has a specific surface area of from about 0.8 to about 4.0 square meters per cubic centimeter. It is preferred that said specific surface area be from about 0.8 to about 3.0 m<sup>2</sup>/c.c. It is more preferred that the specific surface area be from about 0.8 to about 2.4 m<sup>2</sup>/cc. In an even more preferred embodiment, the specific surface area is from about 0.8 to about 2.0 m<sup>2</sup>/cc.

In the slurry produced by the process of this invention, the net zeta potential of the colloidal sized carbonaceous particles in the slurry is from about 15 to about 85 millivolts. The following discussion of zeta potential will refer to a coal-water slurry, it being understood that the discussion is equally applicable to other slurries such as, e.g., a coal-water-oil slurry.

It is preferred that the colloidal sized particles of coal in the coal-water slurry have a net zeta potential of from about 15 to about 85 millivolts. As used herein, the term

"zeta potential" refers to the net potential, be it positive or negative in charge; thus, a zeta potential of from about 15.4 to 70.2 millivolts includes zeta potentials of from about -15.4 to about -70.2 millivolts as well as zeta potentials of from about +15.4 to about +70.2 millivolts. In a more preferred embodiment, said zeta potential is from about 30 to 70 millivolts.

As used in this specification, the term "zeta potential" has the meaning given it in the field of colloid chemistry. Concise discussions and descriptions of the zeta potential and methods for its measurement are found in many sources including, T. M. Riddick, U.S. Pat. No. 3,454,487, issued July, 1969; Douglas et al., U.S. Pat. No. 3,976,582 issued Aug. 24, 1976; *Encyclopedia of Chemistry*, 2nd edition, Clark et al., Reinhold Publ. Corp. 1966, pages 263-265; *Chemical and Process Technology Encyclopedia*, D. M. Considine, editor-in-chief, McGraw-Hill Book Company, N.Y., pages 308-309; *Chemical Technology: An Encyclopedic Treatment*, supra, Vol. VII, pages 27-32; Kirk-Othmer, *Encyclopedia of Chemical Technology*, 2nd Edition, Vol. 22, pages 90-97; and T. M. Riddick, *Control of Colloid Stability Through Zeta Potential*, Zeta-Meter, Inc. New York City. The disclosures of the aforementioned documents are hereby incorporated into this specification by reference.

"Zeta potential" may be measured by conventional techniques and apparatus of electroosmosis such as those described, e.g., in Potter, "Electro Chemistry"; Cleaver-Hume Press, Ltd.; London (1961). Zeta potential can also be determined by measuring electrophoretic mobility (EPM) in any of several commercial apparatuses. In the present invention, a Pen Kem System 3000 (made by Pen Kem Co. Inc. of Bedford Hills, N.Y.) was used for determining zeta potential in the examples herein. This instrument is capable of automatically taking samples of coal particles and producing an EPM distribution by Fast Fourier Transform Analysis from which the average zeta potential can be calculated in millivolts.

40 The zeta potential is measured using very dilute samples of the <10 µm sized coal particles in the coal compact of the coal-water slurry.

It is preferred that the zeta potential of the colloidal sized coal particles in the coal consist of the slurry be negative in charge and be from about -15.4 to about -70.2 millivolts. It is more preferred that said zeta potential be from about -30 to about -70 millivolts.

In one embodiment, it is preferred that the zeta potential of said colloidal sized coal particles be "near maximum". "Near maximum zeta potential", as used in this specification, means a value of zeta potential, measured at constant electrical conductivity, below the maximum zeta potential as defined and discussed in the references cited in the portion of this specification wherein the 55 term "zeta potential" is defined. It is sometimes necessary to normalize the zeta potential values with respect to the electrical conductivity of the carrier fluid because zeta potential is limited by the electrical conductivity of the carrier fluid. The near maximum zeta potential should be of a millivoltage sufficient to provide the coal particles with a repulsive charge great enough to disperse the coal particles in the coal-water slurry. In this embodiment, it is preferred that the zeta potential on the colloidal coal particles be from about 20 to about 60 95 percent of the maximum zeta potential. It is more preferred that the zeta potential on the colloidal coal particles be from about 40 to about 80 percent of the maximum zeta potential for this embodiment.

The maximum zeta potential may be determined by measuring the Brookfield viscosity of the slurry at different zeta potentials. For a given system, maximum zeta potential has been reached when further increases in the surfactant concentration in the slurry do not further decrease the Brookfield viscosity of the system at 100 rpm.

One preferred means for measuring the zeta potential is to grind a sample of coal in either a laboratory size porcelain ball mill with porcelain balls in distilled water at 30 weight percent solids for approximately 24 hours or in a steel ball mill with steel balls at 30 weight percent solids for 16 hours or until all of the particles in the coal are less than 10 microns in size. Small samples of this larger sample can then be prepared in a known way by placing them in a vessel equipped with a stirrer with a sample of water to be used as a carrier in the coal-water slurry. Various acidic and basic salts are then added in incremental amounts to vary the pH, and various concentrations of various candidate dispersing agent or organic surfactants likewise are added in incremental amounts (e.g., grams per gram coal, both dry basis), alone or in combinations of two or more. These samples are then evaluated in any electrophoretic mobility, electroosmosis, or streaming potential apparatus to determine electrical data, from which the zeta potential is calculated in a known way. Plots of zeta potential, pH, and specific conductance vs concentration may then be made to indicate candidate surfactants, or combinations thereof to be used to produce the optimum dispersion of coal particles in the carrier water below the amount at which dilatency may be reached.

Several typical means of producing the slurry are illustrated in FIG. 1. In a wet grinding method, carbonaceous material is charged to crusher 10 and crusher 12. In one embodiment, it is preferred that one carbonaceous material be charged to crusher 10 and another carbonaceous material be charged to crusher 12. In another preferred embodiment, different types of the same carbonaceous material are charged to crushers 10 and 12. In this latter embodiment, the carbonaceous material charged to crushers 10 and 12 can be, e.g., coal, a coal fraction which contains less than about 30 weight percent of volatilizable hydrocarbons (such as, e.g., anthracite or low volatile bituminous coal) can be charged to crusher 10, and a coal fraction which contains more than about 35 weight percent of volatilizable hydrocarbons (such as, e.g., lignite or high volatile bituminous coal) can be charged to crusher 12.

Any of the crushers known to those skilled in the art to be useful for crushing carbonaceous material can be used as crusher 10 and/or crusher 12. The same crusher can be used for crushers 10 or 12, or different crushers can be used. Thus, by way of illustration and not limitation, one can use, e.g., a rod mill, a gyratory crusher, a roll crusher, a jaw crusher, a cage mill, and the like. Generally, the carbonaceous material is crushed to a size of about  $\frac{1}{4} \times 0$ , although coarser and finer fractions can be used.

The crushed material from crusher 10 is fed through line 14. The crushed material from crusher 12 is fed through line 16. Part or all of the crushed material from crusher 10 can be mixed with part or all of the crushed material from crusher 10 by passing the crushed material in line 14 and/or the crushed material in line 16 through transfer line 18. Alternatively, transfer line 18 can be closed, the crushed material from crusher 10 can

be fed directly to mill 26, and the crushed material from crusher 12 can be fed directly to dry grinder 24.

The crushed material from either crusher 10 or 12 can be sampled and measured for pH in the pH meter 13, which will be discussed later, thus establishing a baseline for the entire control circuit discussed later.

The crushed material from crusher 10 can be fed through line 14 to mill 26. Mill 26 can either be a tumbling mill (such as a ball mill, pebble mill, rod mill, tube mill, or compartment mill), or a non-rotary ball or bead mill, such as stirred mills (including the Sweco dispersion mill, the Attritor, the Bureau of Mines mill described in U.S. Pat. No. 3,075,710), vibratory mills such as the Vibro-Energy mill, the Podmore-Boulton mill, the Vibratom, and the like. In general, the various processes and apparatuses which can be used to mill the crushed material are well known to those skilled in the art and are described in e.g., Perry and Chilton's *Chemical Engineer's Handbook*, Fifth Edition (McGraw Hill, New York, 1973) at pages 8-16 to 8-44 (crushing and grinding equipment), the disclosure of which is hereby incorporated by reference into this specification.

In one preferred embodiment, mill 26 is a ball mill which, preferably, is run at a reduced speed. In this embodiment, the mixture is ground at said high solids content of from about 60 to about 82 volume percent of carbonaceous material and at a ball mill speed of from about 50 to about 70 percent of the ball mill critical speed. Thus, for example, the grinding mixture can be ground in a ball mill at a speed of from about 50 to about 70 percent of the ball mill critical speed. The critical speed of the ball mill is the theoretical speed at which the centrifugal force on a ball in contact with the mill shell at the height of its path equals the force on it due to gravity, and it is defined by the equation

$$N_c = 76.6/D$$

wherein  $N_c$  is the critical speed (in rpm), and  $D$  is the diameter of the mill (feet) for a ball diameter that is small with respect to the mill diameter. It is preferred to run ball mill 26 at less than about 60 percent of its critical speed and, more preferably, at less than about 55 percent of its critical speed. The use of reduced critical speed grinding produces a slurry with improved viscosity and stability properties.

In general, mill 26 will have sufficient carbonaceous material and liquid fed to it so that it will contain from about 60 to about 82 volume percent of carbonaceous material. Crushed material is fed to mill 26 through line 14. Alternatively or additionally, milled carbonaceous material (which might or might not contain carrier liquid, such as water) from mill 26 can be recycled through line 40 back into mill 26; this recycled milled carbonaceous material can be either fine milled material which passes through a sieve bend 38 and/or coarser milled material which does not pass through sieve bend 38. Alternatively or additionally, milled carbonaceous material from mill 46 (which preferably contains carrier liquid) can be recycled into mill 26 through lines 48, 58, and 60, or into mill 46 through line 61. Alternatively or additionally, carbonaceous material (which preferably contains carrier liquid) which has been mixed in high shear mixer 64 can be recycled back into mill 26 through lines 66 and 60, or into mill 46 through lines 61.

Carrier liquid is fed to mill 26 through line 20. A sufficient amount of said carrier liquid is fed into the mill 26 so that, in combination with all of the other feeds

to mill 26, a solid-liquid mixture which contains from about 60 to about 82 volume percent of carbonaceous material is produced. The carrier liquid fed to mill 26 is comprised of water and non-aqueous co-liquid. At least about 90 weight percent of said carrier liquid is water, and from about 0.01 to about 10 weight percent of said carrier liquid is non-aqueous liquid.

The mill 26 will have sufficient solids and liquid fed to it so that it will contain from about 60 to about 82 volume percent of solid carbonaceous material. Generally, one should charge from about 0 to about 10 volume percent more solid carbonaceous material to mill 26 than he desires in the final slurry product, subject to the qualification that in no event should more than 82 volume percent of such material be charged to the mill.

Dispersing agent can be added to mill 26 through line 22. For a given material, dispersant, and solids content, a given amount of dispersant will optimize zeta potential; and this amount can be determined in accordance with the screening tests described in this specification. In general, a sufficient amount of dispersant is added through line 22 and/or line 62 and/or line 88 so that the slurry in mill 26 contains from about 0.01 to about 4.0 weight percent of one or more dispersing agents, based on weight of dry carbonaceous material.

A portion of the milled slurry from mill 26 is passed via line 28 through viscometer 30, density meter 32, ph meter 33, and line 27 back to line 28; a portion of the slurry passed to density meter 32 is also passed to particle size distribution analyzer 34. The function of viscometer 30, density meter 32, ph meter 33, and particle size distribution analyzer 34 is to continually monitor the quality of the slurry being produced in mill 26 so that, if necessary, the process can be adjusted by adjusting the feeds of solids and/or solids-fluid slurry and/or liquid and/or dispersant and/or ground carbonaceous material and/or solid-liquid slurry to the mill.

Any of the viscometers known to those skilled in the art can be used as viscometer 30. Thus, by way of illustration, one can use a Nametre Viscometer. The viscometer 30 indicates the viscosity of the ground slurry. If the viscosity of the ground slurry is higher than desired, then either mill 26 is not grinding the coal to produce a sufficiently high surface area and low porosity, and/or the amount or type of dispersing agent used is insufficient to produce a sufficiently high zeta potential on the colloidal carbonaceous particles; and the underflow slurry should be subjected to further tests (in density meter 32, ph meter 33, particle size distribution analyzer 34).

Any of the density meters known to those skilled in the art can be used as density meter 32. Density meter 32 indicates the density of the slurry, which directly varies with its solids content. If the density of the slurry is lower or higher than desired, then it is possible that the particle size distribution of the carbonaceous compact in the underflow slurry is lower or higher than desired. In this case, the slurry should be subjected to further tests in particle size analyzer 34 to determine what the particle size distribution of the underflow slurry is and its attendant surface area and porosity are.

Any ph meters known to those skilled in the art, such as, e.g., Leeds & Northrup in-line ph meter, can be used as ph meter 33. The ph meter measures the hydrogen ion concentration of the slurry, which can vary with water quality, the oxidation state of the carbonaceous or pyrite surfaces, soluble ingredients within the carbonaceous material, or errors in dispersant additions.

Particle size distribution analyzer 34 analyzes the particle size distribution of the compact of the underflow slurry. Any of the particle size distribution analyzers known to those skilled in the art, such as, e.g., Micromeritics Sedigraph 5500L, Coulter Counter, Leeds and Northrup Microtrac Particle Analyzers, can be used as analyzer 34. From the data generated by analyzer 34, the specific surface area and the porosity of the compact of underflow slurry can be determined.

Ground slurry from mill 26 is passed through line 28 to sieve bend 38. Sieve bend 38 may be 40 mesh sieve which, preferably, allows underflow slurry of sufficient fineness (such as, e.g., less than 420 microns) through to line 29 into mill 46 where it is subjected to further grinding; alternatively, all or part of this fine ground slurry can be recycled into mill 26 via line 40. Overflow particles which are greater than 420 microns are recycled via line 40 back into mill 26, where they are subjected to further grinding.

The ground slurry from mill 26 which passes through sieve bend 38 can be passed through line 29 to mill 46. Mill 46 can be a rod mill, a ball mill, or a stirred ball mill; it preferably is a ball mill. It is preferred that the slurry be passed to mill 46 until at least about 95 volume percent of the particles in the slurry have particles less than about 20 microns, and, more preferably, less than about 15 microns; in the most preferred embodiment, the slurry in mill 46 is ground until at least 95 volume percent of the particles in the slurry have diameters less than about 5 microns. Additional liquid and/or dispersant can be added to mill 46 via line 59 if necessary.

A portion of the ground slurry from mill 46 is passed through a control circuit comprised of viscometer 50, density meter 52, and particle size distribution analyzer 54, ph meter 53, and line 56, wherein the slurry is analyzed as described above for the slurry passing from line 28 into viscometer 30, density meter 32, ph meter 33, and particle size distribution analyzer 34. The feed to mill 46 can be adjusted, as required, by feeding crushed carbonaceous material from a dry grinding mill 24 and/or by adjusting the feeds to mill 26.

Slurry from density meter 52 is returned through line 56 to line 48. Part or all of ground slurry from mill 46 can be passed through lines 48, 58, and 60 back to mill 26, wherein it is fed as a recycle stream. Alternatively, or additionally, part or all of ground slurry from mill 46 can be passed via line 61 to mill 46 as a recycle stream. Alternatively, or additionally, part or all of ground slurry from mill 46 can be passed into high shear mixer 64. Any of the high shear, high intensity mixers known to those skilled in the art can be used as high shear mixer 64 and/or high shear mixer 86. Thus, by way of illustration and not limitation, one can use for the high shear mixer(s) a Banbury mixer, a Prodex-Henschel mixer, a Welex-Papenmeir mixer, and the like. These high-shear, intensive mixers are described on page 19-17 of Perry and Chilton's *Chemical Engineer's Handbook*, (McGraw Hill, New York, 1973), the disclosure of which is hereby incorporated by reference into this specification.

Dispersing agent is passed through line 62 to high shear mixer 64 to optimize the zeta potential of the colloidal particles of the slurry in the mixer. A sufficient amount of dispersing agent is charged to this mixer so that the final coal slurry product contains from about 0.01 to about 4.0 weight percent of dispersant, based on the weight of dry coal.

Some or all of the product from high shear mixer 64 can be recycled via lines 66 and 60 to ball mill 26, or via

line 61 to mill 46. Alternatively or additionally, some or all of the product from high shear mixer 64 can be fed through line 68 to hopper 70 and thence to Moyno pump 74 for volumetric blending.

The "Moyno pump", also referred to as a "progressive cavity" or "moving cavity" pump, is well known to those skilled in the art. It consists of a convoluted hardened steel rotor and an inverse convoluted elastomeric stator so designed that as the rotor turns it maintains full contact with the stator on one side and only point to point contact with the stator on the other side. This produces a sealed cavity which moves in the direction of discharge as the rotor turns. Using a variable speed drive this pump can deliver variable volume flow rates at reasonable pressures and at high viscosities. Using a pair of pumps as 74 and 75 allows accurate blending volumetrically of two converging streams of fluids. This is described on pages 19-14 to 19-23 of Perry & Chilton's *Chemical Engineer's Handbook*, 5th edition, supra.

The function of the Moyno pump in the process is to deliver the proper volumetric proportions of two streams from lines 68 and 42 or hoppers 70 and 72 to line 73 to low shear blender 76 via line 73. The blend from blender 76 is then transferred via line 77 using Moyno pump 78 through line 80 to a cleaning apparatus 82.

Material from Moyno pump 74 can be fed through line 73 to low shear blender 76. Any of the low shear blenders known to those skilled in the art can be used. Thus, by way of illustration and not limitation, one can use a twin-blade conical mixer (Atlantic Research Corp.), a double-arm kneader mixer (Baker Perkins Inc.), a helical ribbon mixer, gate mixers, Poly-Eon continuous reactors (Baker Perkins), the Rietz Extructor, Ko-Kneader (Baker Perkins), Transfer mix (Sterling Extruder Corp.), Rotofeed (Baker Perkins), ZSK (Werner-Pfleiderer), Halo-flite Processor (Joy Mfg. Co.), Kneadermaster (Patterson Industries Inc.), etc. Thereafter, the product from low shear blender 76 can be fed through line 77 to Moyno pump 78 and thence through line 80 to cleaner 82.

Cleaned slurry from cleaner 82 can be passed through line 83 to high shear mixer 86. Alternatively, or additionally, cleaner 82 can be bypassed in whole or in part and product from Moyno pump 78 and/or mill 24 can be passed through lines 17 and 84 to high shear mixer 86. Required amounts of dispersant and liquid are fed in lines 88 and 90, respectively to the high shear mixer. A final control circuit, comprised of viscometer 94, density meter 96, particle size distribution analyzer 98, zeta meter 100, ash and sulfur analyzer 102 and pH meter 103, allows one to analyze a portion of the slurry being produced in high shear mixer 86 so that appropriate adjustments can be made in the feeds.

Any of the zeta meters known to those skilled in the art can be used as zeta meter 100. Similarly, any of the ash and sulfur analyzers known to those skilled in the art can be used as analyzer 102.

FIG. 1 also illustrates a dry grinding process for making the slurry. In this process, which may be used separately and/or in conjunction with the wet grinding process, crushed solid carbonaceous material from crusher 12 is passed through line 16 to dry grinder 24; part or all of the material from crusher 12 may alternatively be passed through transfer line 18 to be mixed with solid carbonaceous material from crusher 10 and thence passed through line 14 to mill 26. Any of the dry grinders known to those skilled in the art can be used as

grinder 24. Thus, by way of illustration and not limitation, one can use a hammer mill. Thus, e.g., one can also use ball mills or the ring roller mills described on pages 8-33 and 8-34 or Perry and Chilton's *Chemical Engineer's Handbook*, 5th edition, supra. It is preferred to grind the crushed material in dry grinder 24 until it is pulverized, that is until it is a consist of about 40 mesh by 0.

The pulverized solid carbonaceous material from dry grinder 24 can be passed through line 44 to mill 46 wherein it may be mixed with the feed from line 29 (or, alternatively, not mixed with any such additional feed) and thereafter processed as described hereinabove. Alternatively, or additionally, part or all of the pulverized material from dry grinder 24 can be passed through line 15 and line 14 to mill 26. Alternatively or additionally, part or all of the pulverized carbonaceous material from dry grinder 24 can be passed through line 17 and fed directly into high shear mixer 86, where it is blended with liquid and dispersant and ground to make carbonaceous material-liquid slurry.

In another embodiment, illustrated in FIG. 1 part or all of the underflow slurry which passes through sieve 38 can be passed through line 42 to hopper 72 and thence to Moyno pump 75. The product from Moyno pump 75 is then passed through line 73 to low shear blender 76 and processed as described above.

The operation of the control circuit comprised of viscometer 94, density meter 96, particle size distribution analyzer 98, zeta meter 100, and ash and sulfur analyzer 102 will now be described, it being understood that the other control circuits in the process operate in a similar manner.

In FIG. 1, control circuits are shown which are comprised of a viscometer, a densitometer, a particle size analyzer, and a pH meter. As will be apparent to those skilled in the art, fewer or more such control circuits can be used in the process, and the control circuits can be located at points in the process other than those indicated in FIG. 2.

A typical control circuit is comprised of viscometer 30, densitometer 32, particle size analyzer 34, and pH meter 33. This circuit continually monitors the viscosity, density, consist particle size distribution, and pH of the slurry, and it adjusts the process so that these factors are properly interrelated.

If the density of the slurry is not within the target range, or if the viscosity is too low, then the control circuit determines this and adjusts the ratio of the solids flow rate in the process to the liquids flow rate in the process, thereby adjusting the solids/liquids ratio.

If the viscosity of the slurry is higher than the target range, then the control circuit determines this and adjusts the dispersant concentration (insufficient dispersant can cause a viscosity increase), the solid and/or the liquid flow rate (an insufficient liquid flow rate will cause the solids/liquids ratio to be too high, and will thus cause the viscosity to increase), the pH (if the pH of the grinding mixture is too low, the viscosity might be too high), and/or the particle size distribution. The pH of the grinding mixture can be adjusted by adding more dispersant and/or a pH adjusting agent such as, e.g., caustic. It is to be understood that all of these factors are interrelated, and that the control circuit can, and preferably does, monitor and adjust all of these factors simultaneously.

For any given solids-slurry system, the target particle size distribution can be determined by analyzing "ideal"

slurry and determining its particle size distribution; an "ideal" slurry is one which has the required solids content and viscosity and which fits into the equations described elsewhere in this specification. The particle size distribution of this "ideal slurry" can be determined on two Leeds and Northrup Microtrac Particle Analyzers-the Extended Range Analyzer (300-3  $\mu\text{m}$ ) and the Small Particle Analyzer (21-0.1  $\mu\text{m}$ ). The percent of the particles in the slurry consist which are less than 300 microns, 212 microns, 150 microns, 106 microns, 75 10 microns, 53 microns, 38 microns, 27 microns, etc. can be determined. Then, armed with this particle size profile for the ideal slurry, the particle size analyzer in the control circuit can continually analyze the particle size distribution of the slurry in the process and, if it is less than ideal, the control circuit can adjust the process accordingly. In general, the percent of the particles in the slurry consist which are less than a certain specified particle size can be adjusted by adjusting the relative feed rates of the solids and the liquids fed to the system. For example, if the particle size analyzer indicates that the percent of the particles in the consist less than 212 microns is not within the target range, this can be adjusted by varying the dry carbonaceous material feed rate. For another example, a change in the entire particle size distribution of the slurry consist, including the percent less than 212  $\mu\text{m}$ , can be made by varying the solids/liquids ratio, i.e., by adjusting the volume percent solids in the grinding mixture.

Of particular importance in the particle size distribution analysis is the control of the "n" and the specific surface area of the slurry consist. The "n" in the particle size distribution equation is proportional to the difference between the weight percent concentrations of two selected channels in the Microtrac ER analyzer; the difference between the weight percent concentrations of, e.g., particles less than 150 microns and particles less than 53 microns can be determined for the aforementioned "ideal" slurry; and, armed with this "ideal difference" between said concentrations, the particle size analyzer can continually determine this difference for the slurry in the process and, if it varies from the ideal, the control circuit can adjust the relative feed rates of the solids and liquids fed to the system. The specific surface area of the consist in the slurry is proportional to the difference between the weight percent concentrations of two selected channels in the Microtrac SPA analyzer; the difference between the weight percent of, e.g., particles less than 1.01 and 0.34 microns can be determined for the aforementioned "ideal slurry"; and, armed with this "ideal difference", the particle size analyzer can continually determine this difference for the slurry in the process and, if it varies from the ideal, the control circuit can adjust the relative feed rates of the solids and liquids fed to the system.

The control system described in FIG. 1 is capable, thus, of continually monitoring and adjusting the slurry solids content, the slurry viscosity, the particle size distribution of the slurry consist, the "n" of the slurry consist, and the specific surface area of the slurry consist.

As indicated above, if the viscosity of the slurry is higher than the target rate, the control circuit determines this and can adjust the dispersant concentration and/or the solid flow rate and/or the liquid flow rate and/or the pH. Alternatively, or additionally, the control circuit can adjust the amount of reground carbonaceous fine material being recycled to the grinding mill;

an insufficient amount of colloidally sized carbonaceous material in the slurry consist will cause the viscosity of the slurry to be too high, and the addition of finely ground carbonaceous material to such a slurry tends to reduce its viscosity. For example, if viscometer 30 determines that the slurry in mill 26 is too viscous, it can cause finely ground carbonaceous material from mill 46 and/or high shear mixer 64 to be recycled through line 60 to mill 26, thereby increasing the amount of fine material in the grinding mixture in mill 26 and tending to lower its viscosity. For example, if viscometer 94 determines that the slurry in high shear mixer 86 is too viscous, it can cause finely ground carbonaceous material from mill 46 and/or high shear mixer 64 to be recycled through line 60 to mill 26, thereby increasing the amount of fine material in the slurry ultimately fed to high shear mixer 86 through line 84; it can recycle finely ground carbonaceous material from mill 46 through lines 48, 58, 60, and 61 back into mill 46; it can recycle finely ground carbonaceous material from high shear mixer 64 through lines 66, 58 and 48 back into high shear mixer 64; it can recycle finely ground carbonaceous material from mill 26 through lines 28 and 40 back into mill 26; it can do any combination of the aforementioned steps; and the like. The aforementioned means of increasing the amount of finely ground carbonaceous material in mills 26 and 46 and mixers 64 and 86 are only illustrative, and those skilled in the art upon an examination of FIG. 1 will appreciate other means which can be used.

Thus, the control circuit can adjust the viscosity of the slurry in mill 26 by adjusting the amount of carbonaceous material fed through line 14, the amount of carbonaceous material fed through lines 16 and 18, the amount of carbonaceous material fed through line 15, the amount of carrier liquid fed through line 20, the amount of dispersant fed through line 22, the amount of finely ground carbonaceous material recycled through lines 28 and 40, the amount of finely ground carbonaceous material recycled through lines 48, 58, and 60, the amount of finely ground carbonaceous material recycled through lines 66 and 60, and/or the pH. Thus, the control circuit can adjust the viscosity of the slurry in mill 26 through lines 66 and 60, and/or the pH. Thus, the control circuit can adjust the viscosity of the slurry in mill 46 by adjusting any or all of the aforementioned factors influencing the slurry viscosity in mill 26, (for the properties of the slurry coming out of mill 26 influence the properties of the slurry formed in mill 46), and, additionally or alternatively, the amount of carbonaceous material fed to mill 46 through line 44, and the amount of carbonaceous material fed to mill 46 through line 29. Thus, the control circuit can adjust the viscosity of the slurry in high shear mixer 64 by adjusting any or all of the aforementioned factors influencing the slurry viscosity in mill 26 and 46 (for when the properties of these slurries are changed, they change the properties of the slurry in mixer 64) and, alternatively or additionally, the amount of dispersing agent added through line 62, and the amount of finely ground carbonaceous material recycled through lines 66 and 58 to mixer 64. Thus, the control circuit can adjust the viscosity of the slurry in high shear mixer 86 by adjusting any of the aforementioned factors influencing the slurry viscosity in mill 26, mill 46, and high shear mixer 64, and, alternatively or additionally, the amount of dispersing agent fed to mixer 86 through line 88, the amount of carrier liquid fed to mixer 86 through line 90, the amount of dry car-

bonaceous material fed to high shear mixer through line 17, the amount of finely ground carbonaceous material fed through line 42 to hopper 72, the pH of the slurry in mixer 86, and the like.

Cleaner 82, referred to in FIG. 1, can be any of the 5 carbonaceous-slurry cleaning apparatuses known to those skilled in the art. Thus, by way of illustration and not limitation, one can use the electrophoretic deashing cell illustrated on page 3 (FIG. 3) of Miller and Baker's Bureau of Mines Report of Investigations 7960 (U.S. 10 Department of the Interior, Bureau of Mines, 1974), the disclosure of which is hereby incorporated by reference into this specification. Thus, one can clean said slurry by passing it onto a sedimentation device, such as a lamella filter, where it is allowed to settle. Thus, one 15 can effect magnetic separation of the slurry and/or combine such magnetic separation with sedimentation in the form of a pre- or post-treatment step.

In one preferred embodiment, cleaner 82 involves the 20 cleaning process described in U.S. Pat. Nos. 4,186,887, and 4,173,530, the disclosures of which patents are hereby incorporated by reference into this application. In this preferred embodiment, it is preferred that no 25 dispersing agent be added to the carbonaceous material-fluid mixture until after the mixture has passed through cleaner 82 into high shear mixer 86, at which time the required amount of dispersant is added; thus, in this preferred embodiment, no dispersing agent is added to mill 26.

In one preferred embodiment, the carbonaceous solid 30 material in the grinding mixture (and in the slurry produced therefrom) contains less than about 5 weight percent of ash. The term "ash", as used in this specification, includes non-carbonaceous impurities such as, e.g., inorganic sulfur, various metal sulfides, and other metal 35 impurities as well as soil and clay particles. The fraction of ash in the carbonaceous material can be calculated by dividing the weight of all of the non-carbonaceous material in the slurry solids by the total weight of the slurry solids (which includes both carbonaceous and non-carbonaceous material).

It is preferred that the slurry have a pH from about 5 to about 12 and, preferably, from about 7 to about 11. Conventional means may be used to adjust the pH of the slurry so that it is within these ranges.

In one preferred embodiment, the slurry possesses a unique property; its viscosity decreases at a constant shear rate with time, at an increasing shear rate, and at an increasing temperature; this property greatly enhances the pumpability of the slurry.

In one embodiment, the slurry is a yield-pseudoplastic fluid. The term "yield pseudoplastic fluid", as used in this specification, has the usual meaning associated with it in the field of fluid flow. Specifically, a yield pseudoplastic fluid is one which requires that a yield stress be 55 exceeded before flow commences, and one whose apparent viscosity decreases with increasing rate of shear. In a shear stress vs. shear rate diagram, the curve for a yield pseudoplastic fluid shows a non-linearly increasing shear stress with a linearly increasing rate of shear. In a "pure" pseudoplastic system, no yield stress is observed so that the curve passes through the origin. However, most real systems do exhibit a yield stress, indicating some plasticity. For a yield pseudoplastic fluid, the viscosity decreases with increased shear rate. 65

In an even more preferred embodiment, the slurry produced by the process is also thixotropic, i.e., its viscosity decreases with time at a constant shear rate.

Furthermore, in this embodiment, the slurry has a negative temperature coefficient of viscosity, i.e., its viscosity decreases with increasing temperature.

## EXAMPLE

### Example 1

#### Preparation of Coal Samples for Measurements

##### (a) Sieve analysis

Although any standard procedure may be used to measure particle sizes of coal particles from a coal and then to calculate the particle size distribution, the procedure used in obtaining data discussed herein will be described.

A weighed sample, e.g. 50 grams dry weight of coal is dispersed in 400 m.l. of carrier water containing 1.0 weight % Lomar D based on a weight of coal, dry basis, and the slurry is mixed for 10 minutes with a Hamilton Beach mixer.

The sample is then remixed very briefly. It then is poured slowly on a stack of tared U.S. Standard sieves over a large vessel. The sample is carefully washed with running water through the top sieve with the rest of the stack intact until all sievable material on that sieve is washed through the sieve into the underlying sieves. The top sieve is then removed and each sieve in the stack, as it becomes the top sieve, is successively washed and removed until each sieve has been washed. The sieves are then dried in a dryer at 105° C. and the residue on each is weighed in a known way.

##### (b) Sedigraph analysis

A separate sample finer than 140 mesh sieve size is carefully stirred, and a representative sample (about 200 m.l.) is taken for analysis. The rest may be discarded.

About 2 eyedroppers of the dilute slurry are further diluted in 30 m.l. of distilled water with 4 drops of Lomar D added. This sample is stirred overnight with a magnetic stirrer. Measurement is then made with the Sedigraph 5500L.

The sedigraph 5500L uses photoextinction to measure particles. It essentially measures projected area of shadows, and the data must be converted to volume-%-finer-than. The data from the sieve and Sedigraph is 45 combined to prepare a CPFT chart.  $D_s$  at 1% is read from the CPFT line.

It is to be understood that the foregoing description and Example are illustrative only and that changes can be made in the ingredients and their proportions and in the sequence and combinations of process steps as well as other aspects of the invention discussed without departing from the scope of the invention as defined in the following claims.

I claim:

1. A process for preparing a carbonaceous slurry which is comprised of at least about 60 volume percent of solid carbonaceous material and which has a Brookfield viscosity at a solids content of 70 volume percent, ambient temperature, and ambient pressure, of less than 60 5,000 centipoise, comprising the steps of:

(a) providing a carbonaceous compact, wherein:

1. said compact has a specific surface area of from about 0.8 to about 4.0 square meters per cubic centimeter and an interstitial porosity of less than about 20 volume percent,

2. said compact comprises finely divided solid carbonaceous particles,

3. from about 5 to about 70 weight percent of said solid carbonaceous particles are of colloidal size, being smaller than about 3.0 microns,  
 4. at least about 85 weight percent of said solid carbonaceous particles in the compact have a particle size less than about 300 microns, and  
 5. said compact of finely divided solid carbonaceous particles has a particle size distribution substantially in accordance with the following formula:

$$\frac{CPFT}{100} = \sum_{j=1}^k \left[ X_j \left( \frac{D^{Nj} - D_{sj}^{Nj}}{D_{Lj}^{Nj} - D_{sj}^{Nj}} \right) \right]$$

$$\text{where } \sum_{j=1}^k X_j = 1.0$$

$$\text{and where if } D < D_{sj} \left( \frac{D^{Nj} - D_{sj}^{Nj}}{D_{Lj}^{Nj} - D_{sj}^{Nj}} \right) = 0.0$$

$$\text{and where if } D > D_{Lj} \left( \frac{D^{Nj} - D_{sj}^{Nj}}{D_{Lj}^{Nj} - D_{sj}^{Nj}} \right) = 1.0$$

wherein:

- (a) CPFT is the cumulative percent of said solid carbonaceous material finer than a certain specified particle size D, in volume percent;  
 35 (b) k is the number of component distributions in the consist and is at least 1;  
 (c) X<sub>j</sub> is the fractional amount of the component j in the consist, is less than or equal to 1.0, and the sum of all of the X<sub>j</sub>'s in the consist is 1.0;  
 (d) n is the distribution modulus of fraction j and is greater than about 0.001;  
 (e) D is the diameter of any particle in the consist and ranges from about 0.05 to about 1180 microns;  
 45 (f) D<sub>s</sub> is the diameter of the particle in fraction j, measured at 1% CPFT on a plot of CPFT versus size D, is less than D<sub>L</sub>, and is greater than 0.05 microns;

- (g) D<sub>L</sub> is the diameter of the size modulus in fraction j, measured by sieve size or its equivalent, and is from about 10 to about 1180 microns; and  
 5 (b) mixing from about 60 to about 80 parts, by volume, of said carbonaceous compact with from about 20 to about 40 parts, by volume, of liquid, wherein:  
 1. at least two liquids are mixed with said carbonaceous compact,  
 2. at least about 90 weight percent of the total amount of liquid mixed with said carbonaceous compact is water, and  
 3. from about 0.1 to about 10 weight percent of the total amount of liquid mixed with said carbonaceous compact is non-aqueous liquid.  
 15 2. The process as recited in claim 1, wherein said k is  
 1. 3. The process as recited in claim 2, wherein said non-aqueous liquid is organic liquid.  
 4. The process as recited in claim 3, wherein said carbonaceous material is coal.  
 20 5. The process as recited in claim 4, wherein said non-aqueous liquid is liquid alkane containing from about 5 to about 17 carbon atoms.  
 6. The process as recited in claim 4, wherein said 25 non-aqueous liquid is a liquid petroleum fuel selected from the group consisting of number 1 fuel oil, number 2 fuel oil, number 4 fuel oil, number 5 fuel oil, and number 6 fuel oil.  
 7. The process as recited in claim 6, wherein said 30 non-aqueous liquid is number 2 fuel oil.  
 8. The process as recited in claim 4, wherein said non-aqueous liquid is an aromatic hydrocarbon selected from the group consisting of benzene, toluene, ortho-xylene, meta-xylene, para-xylene, and indene.  
 9. The process as recited in claim 4, wherein said 35 non-aqueous liquid is a nitrogen liquid compound selected from the group consisting of pyridine, alpha-picoline, beta-picoline, gamma-picoline, and quinoline.  
 10. The process as recited in claim 4, wherein said non-aqueous liquid is an oxygen-containing liquid compound selected from the group consisting of ortho-cresol, meta-cresol, and 2,4-dimethylphenol.  
 11. The process as recited in claim 4, wherein said 40 non-aqueous liquid is a liquid monohydric alcohol containing from about 1 to about 18 carbon atoms.  
 12. The process as recited in claim 4, wherein said non-aqueous liquid is a liquid polyhydric alcohol containing from about 2 to about 10 carbon atoms.  
 13. The process as recited in claim 4, wherein said 45 non-aqueous liquid is liquid lubricating oil.

\* \* \* \* \*